



US012342845B2

(12) **United States Patent**  
**Arndt et al.**

(10) **Patent No.:** **US 12,342,845 B2**  
(b4) **Date of Patent:** **Jul. 1, 2025**

(54) **AEROSOL-GENERATING SUBSTRATE  
COMPRISING ZINGIBER SPECIES**

(71) Applicant: **Philip Morris Products S.A.,**  
Neuchatel (CH)

(72) Inventors: **Daniel Arndt**, Neuchatel (CH); **Prisca Campanoni**, Neuchatel (CH);  
**Jean-Pierre Schaller**, Neuchatel (CH)

(73) Assignee: **Philip Morris Products S.A.,**  
Neuchatel (CH)

(\*) Notice: Subject to any disclaimer, the term of this  
patent is extended or adjusted under 35  
U.S.C. 154(b) by 441 days.

(21) Appl. No.: **17/770,493**

(22) PCT Filed: **Oct. 19, 2020**

(86) PCT No.: **PCT/EP2020/079384**  
§ 371 (c)(1),  
(2) Date: **Apr. 20, 2022**

(87) PCT Pub. No.: **WO2021/078691**

PCT Pub. Date: **Apr. 29, 2021**

(65) **Prior Publication Data**

US 2022/0369690 A1 Nov. 24, 2022

(30) **Foreign Application Priority Data**

Oct. 21, 2019 (EP) ..... 19204407

(51) **Int. Cl.**

*A24B 15/167* (2020.01)  
*A24B 3/14* (2006.01)  
*A24B 15/14* (2006.01)  
*A24D 1/18* (2006.01)  
*A24D 1/20* (2020.01)  
*A24F 40/20* (2020.01)

(52) **U.S. Cl.**

CPC ..... *A24B 15/167* (2016.11); *A24B 3/14* (2013.01); *A24B 15/14* (2013.01); *A24D 1/18* (2013.01); *A24D 1/20* (2020.01); *A24F 40/20* (2020.01)

(58) **Field of Classification Search**

CPC ..... A24B 3/14; A24B 15/14; A24B 15/167;  
A24D 1/18; A24D 1/20; A24F 40/20

See application file for complete search history.

(56) **References Cited**

U.S. PATENT DOCUMENTS

|                  |         |                                   |
|------------------|---------|-----------------------------------|
| 3,860,012 A      | 1/1975  | Selke                             |
| 3,894,544 A      | 7/1975  | Egri                              |
| 5,724,998 A      | 3/1998  | Gellatly et al.                   |
| 2012/0055494 A1* | 3/2012  | Hunt ..... A24B 15/186<br>131/111 |
| 2018/0279666 A1* | 10/2018 | Aoun ..... A24B 15/32             |
| 2020/0205463 A1  | 7/2020  | Lamblin et al.                    |
| 2020/0297023 A1  | 9/2020  | Billon et al.                     |

FOREIGN PATENT DOCUMENTS

|    |                    |         |
|----|--------------------|---------|
| CN | 1923064 A          | 3/2007  |
| CN | 101822420 A        | 9/2010  |
| CN | 102160683 A        | 8/2011  |
| CN | 108142982 A        | 6/2018  |
| DE | 10 2015 004 286 A1 | 10/2016 |
| EP | 0 822 760 A2       | 2/1998  |
| EP | 2 793 623 A1       | 10/2014 |
| GB | 983928 A           | 2/1965  |
| JP | 2012-249854 A      | 12/2012 |
| JP | 2017-534266 A      | 11/2017 |
| JP | 6526929 B1         | 6/2019  |
| JP | WO 2019/130500 A1  | 7/2019  |
| JP | WO 2019/189523 A1  | 10/2019 |
| RU | 2 669 151 C1       | 10/2018 |
| WO | WO 95/27411 A1     | 10/1995 |
| WO | WO 2007/010407 A2  | 1/2007  |
| WO | WO 2009/022232 A2  | 2/2009  |
| WO | WO 2011/060961 A1  | 5/2011  |
| WO | WO 2013/034488 A2  | 3/2013  |
| WO | WO 2013/068100 A1  | 5/2013  |
| WO | WO 2013/068304 A1  | 5/2013  |

(Continued)

OTHER PUBLICATIONS

Combined Russian Office Action and Search Report issued Jan. 17, 2024, in corresponding Russian Patent Application No. 2022113496/03(028081) (with English Translation), 13 pages.

Extended European Search Report & Written Opinion issued Apr. 14, 2020 in European Application No. 19204407.1, 7 pages.

Arndt et al., "In-depth characterization of chemical differences between heat-not-burn tobacco products and cigarettes using LC-HRAM-MS-based nontargeted differential screening", 2018, 2 pages (DOI: 10.13140/RG.2.2.11752.16643).

Wachsmuth et al., "Comprehensive chemical characterisation of complex matrices through integration of multiple analytical modes and databases for LC-HRAM-MS-based non-targeted screening", 2018, 2 pages (DOI: 10.13140/RG.2.2.12701.61927).

Buchholz et al., "Increasing confidence for compound identification by fragmentation database and in silico fragmentation comparison with LC-HRAMMS-based non-targeted screening of complex matrices" 2018, 2 pages (DOI: 10.13140/RG.2.2.17944.49927).

(Continued)

*Primary Examiner* — Christopher M Rodd

*Assistant Examiner* — Adam Z Baratz

(74) *Attorney, Agent, or Firm* — Oblon, McClelland, Maier & Neustadt, L.L.P.

(57) **ABSTRACT**

An aerosol-generating article is provided, including: an aerosol-generating substrate including a homogenised ginger material including ginger particles, an aerosol former, and a binder; at least 10 micrograms of [6]-gingerol per gram of the substrate, on a dry weight basis; at least 90 micrograms of [10]-gingerol per gram of the substrate, on a dry weight basis; at least 70 micrograms of [10]-shogaol per gram of the substrate, on a dry weight basis; at least 30 micrograms of [8]-shogaol per gram of the substrate, on a dry weight basis; and at least 80 micrograms of [6]-shogaol per gram of the substrate, on a dry weight basis. An aerosol-generating substrate, an aerosol-generating system, and an aerosol produced upon heating of an aerosol-generating substrate, are also provided.

(56)

**References Cited**

## FOREIGN PATENT DOCUMENTS

|    |                |      |                          |
|----|----------------|------|--------------------------|
| WO | WO 2013/178766 | A1   | 12/2013                  |
| WO | WO 2014/140168 | A2   | 9/2014                   |
| WO | WO 2014/154887 | A1   | 10/2014                  |
| WO | WO 2015/082652 | A1   | 6/2015                   |
| WO | WO 2015/177255 | A1   | 11/2015                  |
| WO | WO-2016184977  | A1 * | 11/2016 ..... A24B 15/14 |
| WO | WO 2017/051034 | A1   | 3/2017                   |
| WO | WO 2017/097840 | A1   | 6/2017                   |
| WO | WO 2019/043119 | A1   | 3/2019                   |
| WO | WO 2019/068930 | A1   | 4/2019                   |
| WO | WO 2020/239597 | A1   | 12/2020                  |

## OTHER PUBLICATIONS

- Arndt et al., "A complex matrix characterization approach, applied to cigarette smoke, that integrates multiple analytical methods and compound identification strategies for non-targeted liquid chromatography with high-resolution mass spectrometry", 12 pages (DOI: 10.1002/rsm.8571).
- Almstetter et al., "Non-targeted screening using GC $\times$ GC-TOFMS for in-depth chemical characterization of aerosol from a heat-not-burn tobacco product", 2018, 2 pages (DOI:10.13140/RG.2.2.36010.31688/1).
- Almstetter et al., "Non-targeted differential screening of complex matrices using GC $\times$ GC-TOFMS for comprehensive characterization of the chemical composition and determination of significant differences" 2016, 2 pages (DOI: 10.13140/RG.2.2.32692.55680).
- Schaller et al., "Evaluation of the Tobacco Heating System 2.2. Part 2: Chemical composition, genotoxicity, cytotoxicity and physical properties of the aerosol," *Regul. Toxicol. and Pharmacol.*, 81 (2016) pp. S27-S47.
- Lee et al., "Antibiofilm and antivirulence activities of 6-gingerol and 6-shogaol against candida albicans due to hyphal inhibition",

Frontiers in Cellular and Infection Microbiology, Aug. 2018, vol. 8, Article 299, 10 pages.

Gopi et al., "Study on temperature dependent conversion of active components of ginger", *International Journal of Pharma Sciences*, vol. 6, No. 1 (2016): 1344-1347 Research Article Open Access, 5 pages.

Schwarner et al., "High-performance liquid chromatographic analysis of 6-gingerol, 8-gingerol, 10-gingerol, and 6-shogaol in ginger-containing dietary supplements, spices, teas, and beverages", *Journal of Chromatography B*, 856, 2007, pp. 41-47.

Jung et al., "Heat-induced conversion of gingerols to shogaols in ginger as affected by heat type (dry or moist heat, sample type (fresh or dried), temperature and time", *Food Science Biotechnology* (2018) 27(3), pp. 687-693, <https://doi.org/10.1007/s10068-017-0301-1>.

Jaapar et al., "Prediction of solubilities for ginger bioactive compounds in hot water by the COSMO-RS method", *Journal of Physics: Conference Series*, 423 (2013) 012066, 11 pagesdoi:10.1088/1742-6596/423/1/012066.

International Search Report issued Feb. 16, 2021 in PCT/EP2020/079384 filed on Oct. 19, 2020, 4 pages.

Written Opinion issued Feb. 16, 2021 in PCT/EP2020/079384 filed on Oct. 19, 2020, 7 pages.

Combined Chinese Office Action and Search Report issued Sep. 20, 2023 in Chinese Application 202080062181.4, (with English translation), 25 pages.

Zhang Junqing et al., "Chinese Medicinal Plants of Zingiberaceous Family", China Medical Science and Technology Press, Dec. 31, 2015, 3 pages.

Combined Chinese Office Action and Search Report issued Feb. 27, 2023, in Chinese Patent Application No. 202080062181.4 (with English translation), 25 pages.

Japanese Office Action issued Oct. 15, 2024 in Japanese Patent Application No. 2022-523518 (with unedited computer-generated English Translation), 5 pages.

\* cited by examiner





Figure 3





Figure 5



Figure 6a



Figure 6b

Figure 6c





Figure 7



Figure 8

**AEROSOL-GENERATING SUBSTRATE  
COMPRISING ZINGIBER SPECIES**

The present invention relates to aerosol-generating substrates comprising homogenised plant material formed from ginger particles and to aerosol-generating articles incorporating such an aerosol-generating substrate. The present invention further relates to an aerosol derived from an aerosol-generating substrate comprising ginger particles.

Aerosol-generating articles in which an aerosol-generating substrate, such as a tobacco-containing substrate, is heated rather than combusted, are known in the art. Typically in such articles, an aerosol is generated by the transfer of heat from a heat source to a physically separate aerosol-generating substrate or material, which may be located in contact with, within, around, or downstream of the heat source. During use of the aerosol-generating article, volatile compounds are released from the substrate by heat transfer from the heat source and are entrained in air drawn through the article. As the released compounds cool, they condense to form an aerosol.

Some aerosol-generating articles comprise a flavourant that is delivered to the consumer during use of the article to provide a different sensory experience to the consumer, for example to enhance the flavour of aerosol. A flavourant can be used to deliver a gustatory sensation (taste), an olfactory sensation (smell), or both a gustatory and an olfactory sensation to the user inhaling the aerosol. It is known to provide heated aerosol-generating articles that include flavourants.

It is also known to provide flavourants in conventional combustible cigarettes, which are smoked by lighting the end of the cigarette opposite the mouthpiece so that the tobacco rod combusts, generating inhalable smoke. One or more flavourants are typically mixed with the tobacco in the tobacco rod in order to provide additional flavour to the mainstream smoke as the tobacco is combusted. Such flavourants can be provided, for example, as essential oil.

Aerosol from a conventional cigarette, which contains a multitude of components interacting with receptors located in the mouth provides a sensation of "mouthfullness," that is to say, a relatively high mouthfeel. "Mouthfeel," as used herein refers to the physical sensations in the mouth caused by food, drink, or aerosol, and is distinct from taste. It is a fundamental sensory attribute which, along with taste and smell, determines the overall flavour of a food item or aerosol.

There are difficulties involved in replicating the consumer experience provided by conventional combustible cigarettes with aerosol-generating articles in which the aerosol-generating substrate is heated rather than combusted. This is partially due to the lower temperatures reached during the heating of such aerosol-generating articles, leading to a different profile of volatile compounds being released.

It would be desirable to provide a novel aerosol-generating substrate for a heated aerosol-generating article providing an aerosol with improved flavour and mouthfullness. It would be particularly desirable if such an aerosol-generating substrate could provide an aerosol with a sensorial experience that is comparable to that provided by a conventional combustible cigarette. It would also be particularly desirable if such an aerosol-generating substrate could provide an aerosol that has reduced levels of undesirable aerosol compounds compared to existing aerosol-generating substrates, for example those containing tobacco only.

It would further be desirable to provide such an aerosol-generating substrate that can be readily incorporated into an

aerosol-generating article and which can be manufactured using existing high-speed methods and apparatus.

The present disclosure relates to an aerosol-generating article comprising an aerosol-generating substrate, the aerosol-generating substrate formed of a homogenised plant material including ginger particles, referred to herein as a "homogenised ginger material". The homogenised ginger material may further comprise an aerosol former. The homogenised ginger material may further comprise a binder.

10 The aerosol-generating substrate may comprise: at least about 10 micrograms of [6]-gingerol per gram of the substrate, on a dry weight basis. The aerosol-generating substrate may comprise at least about 90 micrograms of [10]-gingerol per gram of the substrate, on a dry weight basis. The 15 aerosol-generating substrate may comprise at least about 70 micrograms of [10]-shogaol per gram of the substrate, on a dry weight basis. The aerosol-generating substrate may comprise at least about 30 micrograms of [8]-shogaol per gram of the substrate, on a dry weight basis. The aerosol-generating substrate may comprise at least about 80 micrograms of [6]-shogaol per gram of the substrate, on a dry weight basis.

According to the invention there is provided an aerosol-generating article comprising an aerosol-generating substrate, the aerosol-generating substrate comprising a homogenised plant material including ginger particles. According to the invention, the aerosol-generating substrate comprises: at least about 10 micrograms of [6]-gingerol per gram of the substrate, on a dry weight basis; at least about 90 micrograms of [10]-gingerol per gram of the substrate, on a dry weight basis; at least about 70 micrograms of [10]-shogaol per gram of the substrate, on a dry weight basis; at least about 30 micrograms of [8]-shogaol per gram of the substrate, on a dry weight basis; and at least about 80 micrograms of [6]-shogaol per gram of the substrate, on a dry weight basis.

According to the invention there is provided an aerosol-generating article comprising an aerosol-generating substrate, the aerosol-generating substrate formed of a homogenised ginger material including ginger particles. According to the invention, the homogenised ginger material comprises: ginger particles, an aerosol former and a binder. The aerosol-generating substrate comprises: at least about 10 micrograms of [6]-gingerol per gram of the substrate, on a dry weight basis; at least about 90 micrograms of [10]-gingerol per gram of the substrate, on a dry weight basis; at least about 70 micrograms of [10]-shogaol per gram of the substrate, on a dry weight basis; at least about 30 micrograms of [8]-shogaol per gram of the substrate, on a dry weight basis; and at least about 80 micrograms of [6]-shogaol per gram of the substrate, on a dry weight basis.

Preferably, upon heating of the aerosol-generating substrate of the aerosol-generating article according to the present invention according to Test Method A as described below, an aerosol is generated comprising: at least about 15 micrograms of [6]-gingerol per gram of the substrate, on a dry weight basis; at least about 1.5 micrograms of [10]-gingerol per gram of the substrate, on a dry weight basis; at least about 30 micrograms of [10]-shogaol per gram of the substrate, on a dry weight basis; at least about 15 micrograms of [8]-shogaol per gram of the substrate, on a dry weight basis; and at least about 30 micrograms of [6]-shogaol per gram of the substrate, on a dry weight basis. According to the invention, the amount of [10]-shogaol per gram of the substrate is at least about 10 times the amount of [10]-gingerol per gram of the aerosol-generating substrate.

Preferably, upon heating of the aerosol-generating substrate according to Test Method A, the aerosol generated from the aerosol-generating substrate comprises: [6]-gingerol in an amount of at least about 0.3 micrograms per puff of aerosol; [10]-gingerol in an amount of at least about 0.03 micrograms per puff of aerosol; [10]-shogaol in an amount of at least about 0.7 micrograms per puff of aerosol; [8]-shogaol in an amount of at least about 0.3 micrograms per puff of aerosol; and [6]-shogaol in an amount of at least 0.6 micrograms per puff of aerosol, wherein a puff of aerosol has a volume of 55 millilitres as generated by a smoking machine. According to the invention, the amount of [10]-shogaol per puff is at least about 10 times the amount of [10]-gingerol per puff.

The present disclosure also relates to an aerosol-generating substrate formed of a homogenised plant material comprising ginger particles, referred to herein as "homogenised ginger material". The homogenised ginger material may further comprise an aerosol former. The homogenised ginger material may further comprise a binder. The aerosol-generating substrate may comprise at least about 10 micrograms of [6]-gingerol per gram of the substrate, on a dry weight basis; at least about 90 micrograms of [10]-gingerol per gram of the substrate, on a dry weight basis; at least about 70 micrograms of [10]-shogaol per gram of the substrate, on a dry weight basis; at least about 30 micrograms of [8]-shogaol per gram of the substrate, on a dry weight basis; and at least about 80 micrograms of [6]-shogaol per gram of the substrate, on a dry weight basis.

According to the invention there is also provided an aerosol-generating substrate formed of a homogenised ginger material, wherein the homogenised ginger material comprises ginger particles, an aerosol former and a binder. The aerosol-generating substrate comprises at least about 10 micrograms of [6]-gingerol per gram of the substrate, on a dry weight basis; at least about 90 micrograms of [10]-gingerol per gram of the substrate, on a dry weight basis; at least about 70 micrograms of [10]-shogaol per gram of the substrate, on a dry weight basis; at least about 30 micrograms of [8]-shogaol per gram of the substrate, on a dry weight basis; and at least about 80 micrograms of [6]-shogaol per gram of the substrate, on a dry weight basis.

The present invention further provides an aerosol produced upon heating of an aerosol-generating substrate, the aerosol comprising: [6]-gingerol in an amount of at least about 0.3 micrograms per puff of aerosol; [10]-gingerol in an amount of at least about 0.03 micrograms per puff of aerosol; [10]-shogaol in an amount of at least about 0.7 micrograms per puff of aerosol; [8]-shogaol in an amount of at least about 0.3 micrograms per puff of aerosol; and [6]-shogaol in an amount of at least about 0.6 micrograms per puff of aerosol, wherein a puff of aerosol has a volume of 55 millilitres as generated by a smoking machine of Test Method A. According to the invention, the amount of [10]-shogaol per puff is at least about 10 times the amount of [10]-gingerol per puff.

The present invention further provides a method of making an aerosol-generating substrate comprising: forming a slurry comprising ginger particles, water, an aerosol former, a binder and optionally tobacco particles; casting or extruding the slurry in the form of a sheet or strands; and drying the sheets or strands, preferably at a temperature of between 80 and 160 degrees Celsius. Where a sheet of aerosol-generating substrate is formed, the sheet may optionally be cut into strands or gathered the sheet to form a rod. The sheet may optionally be crimped prior to the gathering step.

Any references below to the aerosol-generating substrates and aerosols of the present invention should be considered to be applicable to all aspects of the invention, unless stated otherwise.

As used herein, the term "aerosol-generating article" refers to an article for producing an aerosol, wherein the article comprises an aerosol-generating substrate that is suitable and intended to be heated or combusted in order to release volatile compounds that can form an aerosol. A conventional cigarette is lit when a user applies a flame to one end of the cigarette and draws air through the other end. The localised heat provided by the flame and the oxygen in the air drawn through the cigarette causes the end of the cigarette to ignite, and the resulting combustion generates an inhalable smoke. By contrast, in "heated aerosol-generating articles", an aerosol is generated by heating an aerosol-generating substrate and not by combusting the aerosol-generating substrate. Known heated aerosol-generating articles include, for example, electrically heated aerosol-generating articles and aerosol-generating articles in which an aerosol is generated by the transfer of heat from a combustible fuel element or heat source to a physically separate aerosol-generating substrate.

Also known are aerosol-generating articles that are adapted to be used in an aerosol-generating system that supplies the aerosol former to the aerosol-generating articles. In such a system, the aerosol-generating substrate in the aerosol-generating articles contain substantially less aerosol former relative to those aerosol-generating substrate which carries and provides substantially all the aerosol former used in forming the aerosol during operation.

As used herein, the term "aerosol-generating substrate" refers to a substrate capable of producing upon heating volatile compounds, which can form an aerosol. The aerosol generated from aerosol-generating substrates may be visible to the human eye or invisible and may include vapours (for example, fine particles of substances, which are in a gaseous state, that are ordinarily liquid or solid at room temperature) as well as gases and liquid droplets of condensed vapours.

As used herein, the term "homogenised plant material" encompasses any plant material formed by the agglomeration of particles of plant. For example, sheets or webs of homogenised plant material for the aerosol-generating substrates of the present invention may be formed by agglomerating particles of plant material obtained by pulverising, grinding or comminuting ginger plant material and optionally tobacco material such as tobacco leaf lamina or tobacco leaf stems. The homogenised plant material may be produced by casting, extrusion, paper making processes or other any other suitable processes known in the art.

As used herein, the term "homogenised ginger material" refers to a homogenised plant material comprising ginger particles, optionally in combination with tobacco particles. The term "homogenised tobacco material" refers to a homogenised plant material comprising tobacco particles but no ginger particles, which is therefore not in accordance with the invention.

As used herein, the term "ginger particles" encompasses particles derived from the dried root of plants of the genus *Zingiber*, preferably particles derived from *Zingiber officinale* Rosc. (Zingiberaceae).

By contrast, ginger essential oil is a distillate produced from ginger by steam distillation and gingerols and shogaols are compounds derived from ginger. These are not considered ginger particles and are not included in the percentages of particulate plant material.

The present invention provides an aerosol-generating article incorporating an aerosol-generating substrate formed of a homogenised plant material including ginger particles, referred to herein as "homogenised ginger material". The present invention also provides an aerosol derived from such an aerosol-generating substrate. The inventors of the present invention have found that through the incorporation of ginger particles into the aerosol-generating substrate, it is advantageously possible to produce an aerosol which provides a novel sensory experience. Such an aerosol provides unique flavours and may provide an increased level of mouthfullness.

In addition, the inventors have found that it is advantageously possible to produce an aerosol with an improved ginger aroma and flavour compared to the aerosol produced through the addition of ginger additives such as ginger oil. Ginger oil is distilled from the root or rhizome of the ginger plant and has a composition of flavourants that are different from ginger particles. This may be at least partially due to the distillation process which may selectively remove or retain certain flavourants. In addition, certain flavour compounds of ginger degrade to form different flavour compounds upon heating or drying of the ginger. The different way in which the ginger oil and ginger plant particles are prepared therefore affects the composition and relative amounts of flavour compounds. For example, upon heating, gingerols are found to degrade to form shogaols and other compounds. The heating and drying of ginger particles in the process of producing an aerosol-forming substrate according to the present invention has been found to increase the level of shogaol compounds present and to decrease the level of gingerol compounds. It is thought that this is due to the conversion of gingerols to shogaols in a dehydration reaction. The resultant change in the relative amounts of gingerols and shogaols has been found to significantly affect the flavour profile of the aerosol produced from the aerosol-generating substrate, relative to an aerosol produced from a ginger oil.

Moreover, in certain aerosol-generating substrates provided herein, ginger particles may be incorporated at a sufficient level to provide the desired ginger flavour whilst maintaining sufficient tobacco material to provide the desired level of nicotine to the consumer.

Furthermore, it has been surprisingly found that the inclusion of ginger particles in an aerosol-generating substrate provides a significant reduction in certain undesirable aerosol compounds compared to an aerosol produced from an aerosol-generating substrate comprising 100 percent tobacco particles without ginger particles.

The flavour released by ginger is due to the presence of one or more volatile flavourants which are volatilised and transferred to the aerosol upon heating. 6-gingerol (5-hydroxy-1-(4-hydroxy-3-methoxyphenyl) decan-3-one, chemical formula:  $C_{17}H_{26}O_4$ ) is the most common chemical constituent found in ginger and provides much of the flavour and aroma.

The presence of ginger in homogenised plant material (such as cast leaf) can be positively identified by DNA barcoding. Methods for performing DNA barcoding based on the nuclear gene ITS2, the rbcL and matK system as well as the plastid intergenic spacer trnH-psbA, are well known in the art and can be used (Chen S, Yao H, Han J, Liu C, Song J, et al. (2010) Validation of the ITS2 Region as a Novel DNA Barcode for Identifying Medicinal Plant Species. PLoS ONE 5(1): e8613; Hollingsworth P M, Graham S W, Little D P (2011) Choosing and Using a Plant DNA Barcode. PLoS ONE 6(5): e19254).

The inventors have carried out a complex analysis and characterisation of the aerosols generated from aerosol-generating substrates of the present invention incorporating ginger particles and a mixture of ginger and tobacco particles, and a comparison of these aerosols with those produced from existing aerosol-generating substrates formed from tobacco material without ginger particles. Based on this, the inventors have been able to identify a group of "characteristic compounds" that are compounds present in the aerosols and which have derived from the ginger particles. The detection of these characteristic compounds within an aerosol within a specific range of weight proportion can therefore be used to identify aerosols that have derived from an aerosol-generating substrate including ginger particles. These characteristic compounds are notably not present in an aerosol generated from tobacco material. Furthermore, the proportion of the characteristic compounds within the aerosol and the ratio of the characteristic compounds to each other are clearly indicative of the use of ginger plant material and not a ginger oil. Similarly, the presence of these characteristic compounds in specific proportions within an aerosol-generating substrate is indicative of the inclusion of ginger particles in the substrate.

In particular, the defined levels of the characteristic compounds within the substrate and the aerosol are specific to the ginger particles present within the homogenised ginger material. The level of each characteristic compound is dependent upon the way in which the ginger particles have been processed during production of the homogenised ginger material. The level is also dependent upon the composition of the homogenised ginger material and in particular, will be affected by the level of other components within the homogenised ginger material. The level of the characteristic compounds within the homogenised ginger material will be different to the level of the same compound within the starting ginger material. It will also be different to the level of the characteristic compounds within materials containing ginger particles but that are not in accordance with the invention as defined herein.

In order to carry out the characterisation of the aerosols, the inventors have made use of complementary non-targeted differential screening (NTDS) using liquid chromatography coupled to high-resolution accurate-mass mass spectrometry (LC-HRAM-MS) in parallel with two-dimensional gas chromatography coupled to time-of-flight mass spectrometry (GCxGC-TOFMS).

Non-targeted screening (NTS) is a key methodology for characterising the chemical composition of complex matrices by either matching unknown detected compound features against spectral databases (suspect screening analysis [SSA]), or if no pre-knowledge matches, by elucidating the structure of unknowns using e.g. first order fragmentation (MS/MS) derived information matched to *in silico* predicted fragments from compound databases (non-targeted analysis [NTA]). It enables the simultaneous measurement and capability for semi-quantification of a large number of small molecules from samples using an unbiased approach.

If the focus is on the comparison of two or more aerosol samples, as described above, to evaluate any significant differences in chemical composition between samples in an unsupervised way or if group related pre-knowledge is available between sample groups, non-targeted differential screening (NTDS) may be performed. A complementary differential screening approach using liquid chromatography coupled to high-resolution accurate-mass mass spectrometry (LC-HRAM-MS) in parallel with two-dimensional gas chromatography coupled to time-of-flight mass spectrometry

(GCxGC-TOFMS) has been applied in order to ensure comprehensive analytical coverage for identifying the most relevant differences in aerosol composition between aerosols derived from articles comprising 100% by weight ginger as the particulate plant material and those derived from articles comprising 100% by weight tobacco as the particulate plant material.

The aerosol was generated and collected using the apparatus and methodology set out in detail below.

LC-HRAM-MS analysis was carried out using a Thermo QExactive™ high resolution mass spectrometer in both full scan mode and data dependent mode. In total, three different methods were applied in order to cover a wide range of substances with different ionization properties and compound classes. Samples were analysed using RP chromatography with heated electrospray ionisation (HESI) in both positive and negative modes and with atmospheric pressure chemical ionisation (APCI) in positive mode. The methods are described in: Arndt, D. et al, "Indepth characterization of chemical differences between heat-not-burn tobacco products and cigarettes using LC-HRAM-MS-based non-targeted differential screening" (DOI:10.13140/RG.2.2.11752.16643); Wachsmuth, C. et al, "Comprehensive chemical characterisation of complex matrices through integration of multiple analytical modes and databases for LC-HRAM-MS-based non-targeted screening" (DOI: 10.13140/RG.2.2.12701.61927); and "Buchholz, C. et al, "Increasing confidence for compound identification by fragmentation database and in silico fragmentation comparison with LC-HRAM-MS-based non-targeted screening of complex matrices" (DOI: 10.13140/RG.2.2.17944.49927), all from the 66th ASMS Conference on Mass Spectrometry and Allied Topics, San Diego, USA (2018). The methods are further described in: Arndt, D. et al, "A complex matrix characterization approach, applied to cigarette smoke, that integrates multiple analytical methods and compound identification strategies for non-targeted liquid chromatography with high-resolution mass spectrometry" (DOI: 10.1002/rclm.8571).

GCxGC-TOFMS analysis was carried out using an Agilent GC Model 6890A or 7890A instrument equipped with an Auto Liquid Injector (Model 7683B) and a Thermal Modulator coupled to a LECO Pegasus 4D™ mass spectrometer with three different methods for nonpolar, polar and highly volatile compounds within the aerosol. The methods are described in: Almstetter et al, "Non-targeted screening using GCxGC-TOFMS for in-depth chemical characterization of aerosol from a heat-not-burn tobacco product" (DOI: 10.13140/RG.2.2.36010.31688/1); and Almstetter et al, "Non-targeted differential screening of complex matrices using GCxGC-TOFMS for comprehensive characterization of the chemical composition and determination of significant differences" (DOI: 10.13140/RG.2.2.32692.55680), from the 66th and 64th ASMS Conferences on Mass Spectrometry and Allied Topics, San Diego, USA, respectively.

The results from the analysis methods provided information regarding the major compounds responsible for the differences in the aerosols generated by such articles. The focus of the non-targeted differential screening using both analytical platforms LC-HRAM-MS and GCxGC-TOFMS was on compounds that were present in greater amounts in the aerosols of a sample of an aerosol-generating substrate according to the invention comprising 100 percent ginger particles relative to a comparative sample of an aerosol-generating substrate comprising 100 percent tobacco particles. The NTDS methodology is described in the papers listed above.

Based on this information, the inventors were able to identify specific compounds within the aerosol that may be considered as "characteristic compounds" deriving from the ginger particles in the substrate. Characteristic compounds unique to ginger include but are not limited to: [10]-shogaol (1-(4-Hydroxy-3-methoxyphenyl)tetradec-4-en-3-one), [8]-shogaol (1-(4-Hydroxy-3-methoxyphenyl)dodec-4-en-3-one), [6]-shogaol (1-(4-Hydroxy-3-methoxyphenyl)dec-4-en-3-one), [6]-gingerol ((S)-5-Hydroxy-1-(4-hydroxy-3-methoxyphenyl)-3-decanone), and [10]-gingerol ((S)-5-Hydroxy-1-(4-hydroxy-3-methoxyphenyl)-3-tetradecanone). For the purposes of the present invention, a targeted screening can be conducted on a sample of aerosol-generating substrate to identify the presence and amount of each of the characteristic compounds in the substrate. Such a targeted screening method is described below. As described, the characteristic compounds can be detected and measured in both the aerosol-generating substrate and the aerosol derived from the aerosol-generating substrate.

As defined above, the aerosol-generating article of the invention comprises an aerosol-generating substrate formed of a homogenised ginger material comprising ginger particles. As a result of the inclusion of the ginger particles, the aerosol-generating substrate comprises certain proportions of the "characteristic compounds" of ginger, as described above. In particular, the aerosol-generating substrate comprises at least about 10 micrograms of [6]-gingerol per gram of the substrate, at least about 90 micrograms of [10]-gingerol per gram of the substrate, at least about 70 micrograms of [10]-shogaol per gram of the substrate, at least about 30 micrograms of [8]-shogaol per gram of the substrate and at least about 80 micrograms of [6]-shogaol per gram of the substrate, on a dry weight basis.

By defining an aerosol-generating substrate with respect to the desired levels of the characteristic compounds, it is possible to ensure consistency between products despite potential differences in the levels of the characteristic compounds in the raw materials. This advantageously enables the quality of the product to be controlled more effectively.

Preferably, the aerosol-generating substrate comprises at least about 100 micrograms of [6]-gingerol per gram of the substrate, more preferably at least about 200 micrograms of [6]-gingerol per gram of the substrate, on a dry weight basis. Alternatively or in addition, the aerosol-generating substrate preferably comprises no more than about 400 micrograms of [6]-gingerol per gram of the substrate, more preferably no more than about 350 micrograms of [6]-gingerol per gram of the substrate and more preferably no more than about 300 micrograms of [6]-gingerol per gram of the substrate. For example, the aerosol-generating substrate may comprise between about 10 micrograms and about 400 micrograms of [6]-gingerol per gram of the substrate, or between about 100 micrograms and about 350 micrograms of [6]-gingerol per gram of the substrate, or between about 200 micrograms and about 300 micrograms of [6]-gingerol per gram of the substrate, on a dry weight basis.

Preferably, the aerosol-generating substrate comprises at least about 1 mg of [10]-gingerol per gram of the substrate, more preferably at least about 2 mg of [10]-gingerol per gram of the substrate, on a dry weight basis. Alternatively or in addition, the aerosol-generating substrate preferably comprises no more than about 4 mg of [10]-gingerol per gram of the substrate, more preferably no more than about 3.5 mg of [10]-gingerol per gram of the substrate and more preferably no more than about 3 mg of [10]-gingerol per gram of the substrate. For example, the aerosol-generating substrate may comprise between about 90 micrograms and about 4 mg

[10]-gingerol per gram of the substrate, or between about 1 mg and about 3.5 mg [10]-gingerol per gram of the substrate, or between about 2 mg and about 3 mg [10]-gingerol per gram of the substrate, on a dry weight basis.

Preferably, the aerosol-generating substrate comprises at least about 0.75 mg of [10]-shogaol per gram of the substrate, more preferably at least about 1.5 mg of [10]-shogaol per gram of the substrate, on a dry weight basis. Alternatively or in addition, the aerosol-generating substrate preferably comprises no more than about 3 mg of [10]-shogaol per gram of the substrate, more preferably no more than about 2.5 mg of [10]-shogaol per gram of the substrate and more preferably no more than about 2 mg of [10]-shogaol per gram of the substrate. For example, the aerosol-generating substrate may comprise between about 70 micrograms and about 3 mg of [10]-shogaol per gram of the substrate, or between about 0.75 mg and about 2.5 mg of [10]-shogaol per gram of the substrate, or between about 1.5 mg and about 2 mg [10]-shogaol per gram of the substrate, on a dry weight basis.

Preferably, the aerosol-generating substrate comprises at least about 0.4 mg of [8]-shogaol per gram of the substrate, more preferably at least about 0.75 mg of [8]-shogaol per gram of the substrate, on a dry weight basis. Alternatively or in addition, the aerosol-generating substrate preferably comprises no more than about 1 mg of [8]-shogaol per gram of the substrate, more preferably no more than about 0.9 mg of [8]-shogaol per gram of the substrate and more preferably no more than about 0.85 mg of [8]-shogaol per gram of the substrate. For example, the aerosol-generating substrate may comprise between about 30 micrograms and about 1 mg of [8]-shogaol per gram of the substrate, or between about 0.4 mg and about 0.9 mg of [8]-shogaol per gram of the substrate, or between about 0.75 mg and about 0.85 mg [8]-shogaol per gram of the substrate, on a dry weight basis.

Preferably, the aerosol-generating substrate comprises at least about 1 mg of [6]-shogaol per gram of the substrate, more preferably at least about 2 mg of [6]-shogaol per gram of the substrate, on a dry weight basis. Alternatively or in addition, the aerosol-generating substrate preferably comprises no more than about 3.5 mg of [6]-shogaol per gram of the substrate, more preferably no more than about 3 mg of [6]-shogaol per gram of the substrate and more preferably no more than about 2.5 mg of [6]-shogaol per gram of the substrate. For example, the aerosol-generating substrate may comprise between about 80 micrograms and about 3.5 mg of [6]-shogaol per gram of the substrate, or between about 1 mg and about 3 mg of [6]-shogaol per gram of the substrate, or between about 2 mg and about 2.5 mg [8]-shogaol per gram of the substrate, on a dry weight basis.

Preferably, the ratio of the characteristic compounds in the aerosol-generating substrate is such that the amount of [6]-shogaol per gram of the substrate is at least 5 times the amount of [6]-gingerol per gram of the substrate, more preferably at least 7.5 times the amount of [6]-gingerol per gram of the substrate, on a dry weight basis. In contrast, ginger oil typically comprises a level of [6]-gingerol that is similar to or higher than the level of [6]-shogaol.

As defined above, the invention also provides an aerosol-generating article that comprises an aerosol-generating substrate formed of a homogenised ginger material comprising ginger particles, wherein upon heating of the aerosol-generating substrate, an aerosol is generated which comprises the "characteristic compounds" of ginger.

For the purposes of the invention, the aerosol-generating substrate is heated according to "Test Method A". In Test Method A, an aerosol-generating article incorporating the

aerosol-generating substrate is heated in a Tobacco Heating System 2.2 holder (THS2.2 holder) under the Health Canada machine-smoking regimen. For the purposes of carrying out Test Method A, the aerosol-generating substrate is provided in an aerosol-generating article that is compatible with the THS2.2 holder.

The Tobacco Heating System 2.2 holder (THS2.2 holder) corresponds to the commercially available IQOS device (Philip Morris Products SA, Switzerland) as described in Smith et al., 2016, *Regul. Toxicol. Pharmacol.* 81 (S2) S82-S92. Aerosol-generating articles for use in conjunction with the IQOS device are also commercially available.

The Health Canada smoking regimen is a well-defined and accepted smoking protocol as defined in Health Canada 2000—Tobacco Products Information Regulations SOR/2000-273, Schedule 2; published by Ministry of Justice Canada. The test method is described in ISO/TR 19478-1: 2014. In a Health Canada smoking test, an aerosol is collected from the sample aerosol-generating substrate over 12 puffs with a puff volume of 55 millimetres, puff duration of 2 seconds and puff interval of 30 seconds, with all ventilation blocked if ventilation is present.

Thus, in the context of the present invention, the expression "upon heating of the aerosol-generating substrate according to Test Method A" means upon heating of the aerosol-generating substrate in a THS2.2 holder under the Health Canada machine-smoking regimen as defined in Health Canada 2000—Tobacco Products Information Regulations SOR/2000-273, Schedule 2; published by Ministry of Justice Canada, the test method being described in ISO/TR 19478-1:2014.

For the purposes of analysis, the aerosol generated from the heating of the aerosol-generating substrate is trapped using suitable apparatus, depending upon the method of analysis that is to be used.

In a suitable method for generating samples for analysis by LC-HRAM-MS, the particulate phase is trapped using a conditioned 44 mm Cambridge glass fibre filter pad (according to ISO 3308) and a filter holder (according to ISO 4387 and ISO 3308). The remaining gas phase is collected downstream from the filter pad using two consecutive micro-impingers (20 mL) containing methanol and internal standard (ISTD) solution (10 mL) each, maintained at -60 degrees Celsius, using a dry ice-isopropanol mixture. The trapped particulate phase and gas phase are then recombined and extracted using the methanol from the micro-impingers, by shaking the sample, vortexing for 5 minutes and centrifuging (4500 g, 5 minutes, 10 degrees Celsius). The resultant extract is diluted with methanol and mixed in an Eppendorf ThermoMixer (5 degrees Celsius, 2000 rpm). Test samples from the extract are analysed by LC-HRAM-MS in combined full scan mode and data dependent fragmentation mode for identification of the characteristic compounds. For the purposes of the invention, LC-HRAM-MS analysis is suitable for the identification and quantification of [6]-gingerol, [10]-gingerol, [8]-shogaol and [10]-shogaol.

Samples for analysis by GCxGC-TOFMS may be generated in a similar way but for GCxGC-TOFMS analysis, different solvents are suitable for extracting and analysing 60 polar compounds, non-polar compounds and volatile compounds separated from whole aerosol.

For non-polar and polar compounds, whole aerosol is collected using a conditioned 44 mm Cambridge glass fibre filter pad (according to ISO 3308) and a filter holder (according to ISO 4387 and ISO 3308), followed by two micro-impingers connected and sealed in series. Each micro-impinger (20 mL) contains 10 mL dichloromethane/

methanol (80:20 v/v) containing internal standard (ISTD) and retention index marker (RIM) compounds. The micro-impingers are maintained at -80 degrees Celsius, using a dry ice-isopropanol mixture. For analysis of the non-polar compounds, the particulate phase of the whole aerosol is extracted from the glass fibre filter pad using the contents of the micro-impingers. Water is added to an aliquot (10 mL) of the resulting extract and the sample is shaken and centrifuged as described above. The dichloromethane layer is separated, dried with sodium sulphate and analysed by GCxGC-TOFMS in full scan mode. For analysis of the polar compounds, the remaining water layer from the non-polar sample preparation described above is used. ISTD and RIM compounds are added to the water layer, which is then directly analysed by GCxGC-TOFMS in full scan mode.

For volatile compounds, whole aerosol is collected using two micro-impingers (20 mL) connected and sealed in series, each filled with 10 mL N,N-dimethylformamide (DMF) containing ISTD and RIM compounds. The micro-impingers are maintained at between -50 and -60 degrees Celsius using a dry ice-isopropanol mixture. After collection, the contents of the two micro-impingers are combined and analysed by GCxGC-TOFMS in full scan mode.

For the purposes of the invention, GCxGC-TOFMS analysis is suitable for the identification and quantification of [6]-shogaol.

The aerosol generated upon heating of the aerosol-generating substrate of the invention according to Test Method A is characterised by the amounts and ratios of the characteristic compounds, [6]-gingerol, [10]-gingerol, [10]-shogaol, [8]-shogaol and [6]-shogaol, as defined above.

Preferably, in an aerosol-generating article comprising an aerosol-generating substrate as described above, upon heating the aerosol-generating substrate according to Test Method A, an aerosol is generated comprising at least 15 micrograms of [6]-gingerol per gram of the aerosol-generating substrate, at least 90 micrograms of [10]-gingerol per gram of the aerosol-generating substrate, at least 70 micrograms of [10]-shogaol, at least 30 micrograms of [8]-shogaol and at least 80 micrograms of [6]-shogaol per gram of aerosol-generating substrate, on a dry weight basis.

The ranges define the amount of each of the characteristic compounds in the aerosol generated per gram of the aerosol-generating substrate (also referred to herein as the "substrate"). This equates to the total amount of the characteristic compound measured in the aerosol collected during Test Method A, divided by the dry weight of the aerosol-generating substrate prior to heating.

Upon heating of the aerosol-generating substrate according to the present invention according to Test Method A, an aerosol is generated that preferably comprises at least about 200 micrograms of [6]-gingerol per gram of the substrate, more preferably at least about 300 micrograms of [6]-gingerol per gram of the substrate. Alternatively, or in addition, the aerosol generated from the aerosol-generating substrate comprises up to about 750 micrograms of [6]-gingerol per gram of the substrate, preferably up to about 600 micrograms of [6]-gingerol per gram of the substrate and more preferably up to about 450 micrograms of [6]-gingerol per gram of the substrate. For example, the aerosol generated from the aerosol-generating substrate may comprise between about 15 micrograms and about 750 micrograms of [6]-gingerol per gram of the substrate, or between about 200 micrograms and about 600 micrograms of [6]-gingerol per gram of the substrate, or between about 300 micrograms and about 450 micrograms of [6]-gingerol per gram of the substrate.

Upon heating of the aerosol-generating substrate according to the present invention according to Test Method A, an aerosol is generated that preferably comprises at least about 20 micrograms of [10]-gingerol per gram of the substrate, more preferably at least about 30 micrograms of [10]-gingerol per gram of the substrate. Alternatively, or in addition, the aerosol generated from the aerosol-generating substrate comprises up to about 75 micrograms of [10]-gingerol per gram of the substrate, preferably up to about 60 micrograms of [10]-gingerol per gram of the substrate and more preferably up to about 45 micrograms of [10]-gingerol per gram of the substrate. For example, the aerosol generated from the aerosol-generating substrate may comprise between about 1.5 micrograms and about 75 micrograms of [6]-gingerol per gram of the substrate, or between about 20 micrograms and about 60 micrograms of [6]-gingerol per gram of the substrate, or between about 30 micrograms and about 45 micrograms of [6]-gingerol per gram of the substrate.

Upon heating of the aerosol-generating substrate according to the present invention according to Test Method A, an aerosol is generated that preferably comprises at least about 250 micrograms of [10]-shogaol per gram of the substrate, more preferably at least about 500 micrograms of [10]-shogaol per gram of the substrate. Alternatively, or in addition, the aerosol generated from the aerosol-generating substrate comprises up to about 1500 micrograms of [10]-shogaol per gram of the substrate, preferably up to about 1200 micrograms of [10]-shogaol per gram of the substrate and more preferably up to about 1000 micrograms of [10]-shogaol per gram of the substrate. For example, the aerosol generated from the aerosol-generating substrate may comprise between about 30 micrograms and about 1500 micrograms of [10]-shogaol per gram of the substrate, or between about 250 micrograms and about 1200 micrograms of [10]-shogaol per gram of the substrate, or between about 500 micrograms and about 1000 micrograms of [10]-shogaol per gram of the substrate.

Upon heating of the aerosol-generating substrate according to the present invention according to Test Method A, an aerosol is generated that preferably comprises at least about 150 micrograms of [8]-shogaol per gram of the substrate, more preferably at least about 250 micrograms of [8]-shogaol per gram of the substrate. Alternatively, or in addition, the aerosol generated from the aerosol-generating substrate comprises up to about 750 micrograms of [8]-shogaol per gram of the substrate, preferably up to about 600 micrograms of [8]-shogaol per gram of the substrate and more preferably up to about 500 micrograms of [8]-shogaol per gram of the substrate. For example, the aerosol generated from the aerosol-generating substrate may comprise between about 15 micrograms and about 750 micrograms of [8]-shogaol per gram of the substrate, or between about 150 micrograms and about 600 micrograms of [8]-shogaol per gram of the substrate, or between about 250 micrograms and about 500 micrograms of [8]-shogaol per gram of the substrate.

Upon heating of the aerosol-generating substrate according to the present invention according to Test Method A, an aerosol is generated that preferably comprises at least about 250 micrograms of [6]-shogaol per gram of the substrate, more preferably at least about 500 micrograms of [6]-shogaol per gram of the substrate. Alternatively, or in addition, the aerosol generated from the aerosol-generating substrate comprises up to about 1500 micrograms of [6]-shogaol per gram of the substrate, preferably up to about 1200 micrograms of [6]-shogaol per gram of the substrate

and more preferably up to about 1000 micrograms of [6]-shogaol per gram of the substrate. For example, the aerosol generated from the aerosol-generating substrate may comprise between about 30 micrograms and about 1500 micrograms of [6]-shogaol per gram of the substrate, or between about 250 micrograms and about 1200 micrograms of [6]-shogaol per gram of the substrate, or between about 500 micrograms and about 1000 micrograms of [6]-shogaol per gram of the substrate.

Preferably, the aerosol generated from the aerosol-generating substrate during Test Method A has an amount of [10]-shogaol per gram of the substrate that is at least about 10 times the amount of [10]-gingerol per gram of the substrate. The ratio of [10]-shogaol to [10]-gingerol is therefore at least 10:1.

Preferably, the amount of [10]-shogaol per gram of the substrate is at least about 15 times the amount of [10]-gingerol per gram of the substrate, such that the ratio of [10]-shogaol to [10]-gingerol is at least 15:1. More preferably, the amount of [10]-shogaol per gram of the substrate is at least about 20 times the amount of [10]-gingerol per gram of the substrate, such that the ratio of [10]-shogaol to [10]-gingerol is at least 20:1.

The defined ratio of [10]-shogaol to [10]-gingerol characterises an aerosol that is derived from ginger particles. In contrast, in an aerosol produced from ginger oil, the ratio of [10]-shogaol to [10]-gingerol would be significantly different. This is due to the relatively high proportion of [10]-gingerol in ginger oil whilst the level of [10]-shogaol is at or close to zero.

Preferably, the aerosol produced from an aerosol-generating substrate according to the present invention during Test Method A further comprises at least about 0.1 micrograms of nicotine per gram of the substrate, more preferably at least about 1 microgram of nicotine per gram of the substrate, more preferably at least about 2 micrograms of nicotine per gram of the substrate. Preferably, the aerosol comprises up to about 10 micrograms of nicotine per gram of the substrate, more preferably up to about 7.5 micrograms of nicotine per gram of the substrate, more preferably up to about 4 micrograms of nicotine per gram of the substrate. For example, the aerosol may comprise between about 0.1 micrograms and about 10 micrograms of nicotine per gram of the substrate, or between about 1 microgram and about 7.5 micrograms of nicotine per gram of the substrate, or between about 2 micrograms and about 4 micrograms of nicotine per gram of the substrate. In some embodiments of the present invention, the aerosol may contain zero micrograms of nicotine.

Various methods known in the art can be applied to measure the amount of nicotine in the aerosol.

Alternatively or in addition, the aerosol produced from an aerosol-generating substrate according to the present invention during Test Method A may optionally further comprise at least about 20 milligrams of a cannabinoid compound per gram of the substrate, more preferably at least about 50 milligrams of a cannabinoid compound per gram of the substrate, more preferably at least about 100 milligrams of a cannabinoid compound per gram of the substrate. Preferably, the aerosol comprises up to about 250 milligrams of a cannabinoid compound per gram of the substrate, more preferably up to about 200 milligrams of a cannabinoid compound per gram of the substrate, more preferably up to about 150 milligrams of a cannabinoid compound per gram of the substrate. For example, the aerosol may comprise between about 20 milligrams and about 250 milligrams of a cannabinoid compound per gram of the substrate, or

between about 50 milligrams and about 200 milligrams of a cannabinoid compound per gram of the substrate, or between about 100 milligrams and about 150 milligrams of a cannabinoid compound per gram of the substrate. In some embodiments of the present invention, the aerosol may contain zero micrograms of cannabinoid compound.

Preferably, the cannabinoid compound is selected from CBD and THC. More preferably, the cannabinoid compound is CBD.

Various methods known in the art can be applied to measure the amount of a cannabinoid compound in the aerosol.

Carbon monoxide may also be present in the aerosol generated from an aerosol-generating substrate according to the invention during Test Method A and may be measured and used to further characterise the aerosol. Oxides of nitrogen such as nitric oxide and nitrogen dioxide may also be present in the aerosol and may be measured and used to further characterise the aerosol.

The aerosol produced from an aerosol-generating substrate according to the invention during Test Method A may further comprise at least about 5 milligrams of aerosol former per gram of aerosol-generating substrate, or at least about 10 milligrams of aerosol per gram of the substrate or at least about 15 milligrams of aerosol former per gram of the substrate. Alternatively or in addition, the aerosol may comprise up to about 30 milligrams of aerosol former per gram of the substrate, or up to about 25 milligrams aerosol former per gram of the substrate, or up to about 20 milligrams aerosol former per gram of the substrate. For example, the aerosol may comprise between about 5 milligrams and about 30 milligrams of aerosol former per gram of the substrate, or between about 10 milligrams and about 25 milligrams of aerosol former per gram of the substrate, or between about 15 milligrams and about 20 milligrams of aerosol former per gram of the substrate. In alternative embodiments, the aerosol may comprise less than 5 milligrams of aerosol former per gram of substrate. This may be appropriate, for example, if an aerosol former is provided separately within the aerosol-generating article or aerosol-generating device.

Suitable aerosol formers for use in the present invention are set out below.

Various methods known in the art can be applied to measure the amount of aerosol former in the aerosol.

As described above, the presence of the characteristic compounds in the aerosol in the amounts and ratios defined is indicative of the inclusion of ginger particles in the homogenised ginger material forming the aerosol-generating substrate.

Preferably, the ginger particles comprise at least about 0.1 percent by weight of volatile oils, more preferably at least about 0.2 percent by weight volatile oils and most preferably at least about 0.5 percent by weight of volatile oils, on a dry weight basis. The volatile oil content of the ginger particles can be determined using steam distillation, as set out in ISO 6571:2008. This gives an indication of the essential oil content of the ginger particles.

Preferably, the aerosol-generating substrate according to the invention comprises homogenised ginger material comprising at least about 2.5 percent by weight of ginger particles, on a dry weight basis. Preferably, the particulate plant material comprises at least about 3 percent by weight of ginger particles, more preferably at least about 4 percent by weight of ginger particles, more preferably at least about 5 percent by weight of ginger particles, more preferably at least about 6 percent by weight of ginger particles, more

preferably at least about 7 percent by weight of ginger particles, more preferably at least about 8 percent by weight of ginger particles, more preferably at least about 9 percent by weight of ginger particles, more preferably at least about 10 percent by weight of ginger particles, more preferably at least about 11 percent by weight of ginger particles, more preferably at least about 12 percent by weight of ginger particles, more preferably at least about 13 percent by weight of ginger particles, more preferably at least about 14 percent by weight of ginger particles, more preferably at least about 15 percent by weight of ginger particles, more preferably at least about 20 percent by weight of ginger particles, more preferably at least about 30 percent by weight of ginger particles, on a dry weight basis.

In certain embodiments of the invention, the plant particles forming the homogenised ginger material may include at least 98 percent by weight of ginger particles or at least 95 percent by weight of ginger particles, based on dry weight of the plant particles. In such embodiments, the aerosol-generating substrate therefore comprises ginger particles, with substantially no other plant particles. For example, the plant particles forming the homogenised ginger material may comprise about 100 percent by weight of ginger particles.

In alternative embodiments of the invention, the homogenised ginger material may comprise ginger particles in combination with at least one of tobacco particles or cannabis particles, as described below.

In the following description of the invention, the term "particulate plant material" is used to refer collectively to the particles of plant material that are used to form the homogenised plant material. The particulate plant material may consist substantially of ginger particles or may be a mixture of ginger particles with tobacco particles, cannabis particles, or both tobacco particles and cannabis particles.

The homogenised ginger material may comprise up to about 95 percent by weight of ginger particles, on a dry weight basis. Preferably, the homogenised ginger material comprises up to about 90 percent by weight of ginger particles, more preferably up to about 80 percent by weight of ginger particles, more preferably up to about 70 percent by weight of ginger particles, more preferably up to about 60 percent by weight of ginger particles, more preferably up to about 50 percent by weight of ginger particles, on a dry weight basis.

For example, the homogenised ginger material may comprise between about 2.5 percent and about 95 percent by weight of ginger particles, or about 5 percent and about 90 percent by weight of ginger particles, or between about 10 percent and about 80 percent by weight of ginger particles, or between about 15 percent and about 70 percent by weight of ginger particles, or between about 20 percent and about 60 percent by weight of ginger particles, or between about 30 percent and about 50 percent by weight of ginger particles, on a dry weight basis.

As described above, the inventors have identified a number of "characteristic compounds", which are compounds that are characteristic of the ginger plant and are therefore indicative of the inclusion of ginger plant particles within the aerosol-generating substrate.

The amounts of the characteristic compounds present in pure ginger particles are expected to be different from the amounts that are present in the aerosol-generating substrate. The process of making the substrate, which involves hydration in a slurry or suspension, and drying at elevated temperatures, as well as the presence of other ingredients, such as aerosol former, will differentially modify the

amounts of each of the characteristic compounds. The integrity of the ginger particles and the stability of a compound, under the temperature and subject to the manipulations during the manufacturing will also affect the final amount of the compound that is present in a substrate. It is therefore contemplated that the ratio of the characteristic compounds relative to each other would be different after the ginger particles are incorporated into a substrate in various physical forms, e.g., sheets, strands and granules.

The presence of ginger within an aerosol-generating substrate and the proportion of ginger provided within an aerosol-generating substrate can be determined by measuring the amount of the characteristic compounds within the substrate and comparing this to the corresponding amount of the characteristic compound in pure ginger material. The presence and amount of the characteristic compounds can be conducted using any suitable techniques, which would be known to the skilled person.

In a suitable technique, a sample of 250 milligrams of the aerosol-generating substrate is mixed with 5 millilitres of methanol and extracted by shaking, vortexing for 5 minutes and centrifuging (4500 g, 5 minutes, 10 degrees Celsius). Aliquots (300 microlitres) of the extract are transferred into a silanised chromatographic vial and diluted with methanol (600 microlitres) and internal standard (ISTD) solution (100 microlitres). The vials are closed and mixed for 5 minutes using an Eppendorf ThermoMixer (5 degrees Celsius; 2000 rpm). Test samples from the resultant extract are analysed by LC-HRAM-MS in combined full scan mode and data dependent fragmentation mode for identification of the characteristic compounds.

In some embodiments, the homogenised ginger material further comprises up to about 92 percent by weight of tobacco particles, on a dry weight basis.

For example, the homogenised ginger material preferably comprises between about 10 percent and about 92 percent by weight tobacco particles, more preferably between about 20 percent and about 90 percent by weight tobacco particles, more preferably between about 30 percent and about 85 percent by weight tobacco particles, more preferably between about 40 percent and about 80 percent by weight tobacco particles, more preferably between about 50 percent and about 70 percent by weight tobacco particles, on a dry weight basis.

In some preferred embodiments, the homogenised ginger material comprises between about 5 percent and about 20 percent by weight of ginger particles and between about 55 percent and about 70 percent by weight of tobacco particles, on a dry weight basis.

The weight ratio of the ginger particles and the tobacco particles in the particulate plant material forming the homogenised ginger material may vary depending on the desired flavour characteristics and composition of the aerosol. Preferably, the homogenised ginger material comprises a weight ratio of ginger particles to tobacco particles that is no more than about 1:4. This means that the ginger particles account for no more than 20 percent of the total particulate plant material. More preferably the homogenised ginger material comprises a weight ratio of ginger particles to tobacco particles that is no more than 1:5 and more preferably no more than 1:6.

For example, in a first preferred embodiment, the ratio by weight of ginger particles to tobacco particles is 1:4. A 1:4 ratio corresponds to a particulate plant material consisting of about 20 percent by weight ginger particles and about 80 percent by weight tobacco particles. For homogenised ginger material formed with about 75 percent by weight of

particulate plant material, this corresponds to about 15 percent by weight of ginger particles and about 60 percent by weight of tobacco particles in the homogenised ginger material, based on dry weight.

In another embodiment, the homogenised ginger material comprises a 1:9 weight ratio of ginger particles to tobacco particles. In yet another embodiment, the homogenised ginger material comprises a 1:30 weight ratio of ginger particles to tobacco particles.

With reference to the present invention, the term "tobacco particles" describes particles of any plant member of the genus *Nicotiana*. The term "tobacco particles" encompasses ground or powdered tobacco leaf lamina, ground or powdered tobacco leaf stems, tobacco dust, tobacco fines, and other particulate tobacco by-products formed during the treating, handling and shipping of tobacco. In a preferred embodiment, the tobacco particles are substantially all derived from tobacco leaf lamina. By contrast, isolated nicotine and nicotine salts are compounds derived from tobacco but are not considered tobacco particles for purposes of the invention and are not included in the percentage of particulate plant material.

The tobacco particles may be prepared from one or more varieties of tobacco plants. Any type of tobacco may be used in a blend. Examples of tobacco types that may be used include, but are not limited to, sun-cured tobacco, flue-cured tobacco, Burley tobacco, Maryland tobacco, Oriental tobacco, Virginia tobacco, and other speciality tobaccos.

Flue-curing is a method of curing tobacco, which is particularly used with Virginia tobaccos. During the flue-curing process, heated air is circulated through densely packed tobacco. During a first stage, the tobacco leaves turn yellow and wilt. During a second stage, the laminae of the leaves are completely dried. During a third stage, the leaf stems are completely dried.

Burley tobacco plays a significant role in many tobacco blends. Burley tobacco has a distinctive flavour and aroma and also has an ability to absorb large amounts of casing.

Oriental is a type of tobacco which has small leaves, and high aromatic qualities. However, Oriental tobacco has a milder flavour than, for example, Burley. Generally, therefore, Oriental tobacco is used in relatively small proportions in tobacco blends.

Kasturi, Madura and Jatim are subtypes of sun-cured tobacco that can be used. Preferably, Kasturi tobacco and flue-cured tobacco may be used in a blend to produce the tobacco particles. Accordingly, the tobacco particles in the particulate plant material may comprise a blend of Kasturi tobacco and flue-cured tobacco.

The tobacco particles may have a nicotine content of at least about 2.5 percent by weight, based on dry weight. More preferably, the tobacco particles may have a nicotine content of at least about 3 percent, even more preferably at least about 3.2 percent, even more preferably at least about 3.5 percent, most preferably at least about 4 percent by weight, based on dry weight. When the aerosol-generating substrate contains tobacco particles in combination with ginger particles, tobaccos having a higher nicotine content are preferred to maintain similar levels of nicotine relative to typical aerosol-generating substrates without ginger particles, since the total amount of nicotine would otherwise be reduced due to substitution of tobacco particles with ginger particles.

As a result of the inclusion of the tobacco particles, the aerosol-generating substrate and the aerosol generated from the aerosol-generating substrate of such embodiments comprise certain proportions of the "characteristic compounds"

of tobacco. Characteristic compounds generated from tobacco include but are not limited to anatabine, cotinine, and damascenone.

Nicotine may optionally be incorporated into the aerosol-generating substrate although this would be considered as a non-tobacco material for the purposes of the invention. The nicotine may comprise one or more nicotine salts selected from the list consisting of nicotine lactate, nicotine citrate, nicotine pyruvate, nicotine bitartrate, nicotine benzoate, nicotine pectate, nicotine alginate, and nicotine salicylate. Nicotine may be incorporated in addition to a tobacco with low nicotine content, or nicotine may be incorporated into an aerosol-generating substrate that has a reduced or zero tobacco content.

In certain embodiments of the invention, the aerosol-generating substrate comprises a homogenised ginger material formed from particulate plant material consisting of ginger particles only, with nicotine, such as a nicotine salt, incorporated into the aerosol-generating substrate.

Preferably, the aerosol-generating substrate comprises at least about 0.1 mg of nicotine per gram of the substrate, on a dry weight basis. More preferably, the aerosol-generating substrate comprise at least about 0.5 mg of nicotine per gram of the substrate, more preferably at least about 1 mg of nicotine per gram of the substrate, more preferably at least about 1.5 mg of nicotine per gram of the substrate, more preferably at least about 2 mg of nicotine per gram of the substrate, more preferably at least about 3 mg of nicotine per gram of the substrate, more preferably at least about 4 mg of nicotine per gram of the substrate, more preferably at least about 5 mg of nicotine per gram of the substrate, on a dry weight basis.

Preferably, the aerosol-generating substrate comprises up to about 50 mg of nicotine per gram of the substrate, on a dry weight basis. More preferably, the aerosol-generating substrate comprises up to about 45 mg of nicotine per gram of the substrate, more preferably up to about 40 mg of nicotine per gram of the substrate, more preferably up to about 35 mg of nicotine per gram of the substrate, more preferably up to about 30 mg of nicotine per gram of the substrate, more preferably up to about 25 mg of nicotine per gram of the substrate, more preferably up to about 20 mg of nicotine per gram of the substrate, on a dry weight basis.

For example, the aerosol-generating substrate may comprise between about 0.1 mg and about 50 mg of nicotine per gram of the substrate, or between about 0.5 mg and about 45 mg of nicotine per gram of the substrate, or between about 1 mg and about 40 mg of nicotine per gram of the substrate, or between about 2 mg and about 35 mg of nicotine per gram of the substrate, or between about 5 mg and about 30 mg of nicotine per gram of the substrate, or between about 10 mg and about 25 mg of nicotine per gram of the substrate, or between about 15 mg and about 20 mg of nicotine per gram of the substrate, on a dry weight basis. In certain preferred embodiments of the invention, the aerosol-generating substrate comprises between about 1 mg and about 20 mg of nicotine per gram of the substrate, on a dry weight basis.

The defined ranges of nicotine content for the aerosol-generating substrate include all forms of nicotine which may be present in the aerosol-generating substrate, including nicotine intrinsically present in tobacco material as well as nicotine that has been optionally added separately to the aerosol-generating substrate, for example, in the form of a nicotine salt.

Alternatively or in addition to the inclusion of tobacco particles into the homogenised ginger material of the aerosol-generating substrate according to the invention, the

homogenised ginger material may comprise up to 92 percent by weight of cannabis particles, on a dry weight basis. The term "cannabis particles" refers to particles of a cannabis plant, such as the species *Cannabis sativa*, *Cannabis indica*, and *Cannabis ruderalis*.

For example, the particulate plant material may comprise between about 10 percent and about 92 percent by weight of cannabis particles, more preferably between about 20 percent and about 90 percent by weight tobacco particles, more preferably between about 30 percent and about 85 percent by weight tobacco particles, more preferably between about 40 percent and about 80 percent by weight tobacco particles, more preferably between about 50 percent and about 70 percent by weight tobacco particles, on a dry weight basis.

One or more cannabinoid compounds may optionally be incorporated into the aerosol-generating substrate although this would be considered as a non-cannabis material for the purposes of the invention. As used herein with reference to the invention, the term "cannabinoid compound" describes any one of a class of naturally occurring compounds that are found in parts of the cannabis plant—namely the species *Cannabis sativa*, *Cannabis indica*, and *Cannabis ruderalis*. Cannabinoid compounds are especially concentrated in the female flower heads and commonly sold as cannabis oil. Cannabinoid compounds naturally occurring in the cannabis plant include tetrahydrocannabinol (THC) and cannabidiol (CBD). In the context of the present invention, the term "cannabinoid compounds" is used to describe both naturally derived cannabinoid compounds and synthetically manufactured cannabinoid compounds.

For example, the aerosol-generating substrate may comprise a cannabinoid compound selected from the group consisting of: tetrahydrocannabinol (THC), tetrahydrocannabinolic acid (THCA), cannabidiol (CBD), cannabidiolic acid (CBDA), cannabinol (CBN), cannabigerol (CBG), cannabigerol monomethyl ether (CBGM), cannabivarin (CBV), cannabidivarin (CBDV), tetrahydrocannabivarin (THCV), cannabichromene (CBC), cannabicyclol (CBL), cannabichromevarin (CBCV), cannabigerovarin (CBGV), cannabielsin (CBE), cannabicitran (CBT) and combinations thereof.

The homogenised ginger material may further comprise a proportion of other plant flavour particles in addition to the ginger particles or the combination of ginger particles with at least one of tobacco particles and cannabis particles (the "particulate plant material").

For the purposes of the present invention, the term "other plant flavour particles" refers to particles of non-ginger, non-tobacco and non-cannabis plant material, that are capable of generating one or more flavourants upon heating. This term should be considered to exclude particles of inert plant material such as cellulose, that do not contribute to the sensory output of the aerosol-generating substrate. The particles may be derived from ground or powdered leaf lamina, fruits, stalks, stems, roots, seeds, buds or bark from the other plants. Suitable plant flavour particles for inclusion in an aerosol-generating substrate according to the invention would be known to the skilled person and include but are not limited to clove particles and tea particles.

The composition of the homogenised ginger material can advantageously be adjusted through the blending of desired amounts and types of the different plant particles. This enables an aerosol-generating substrate to be formed from a single homogenised ginger material, if desired, without the need for the combination or mixing of different blends, as is the case for example in the production of conventional cut

filler. The production of the aerosol-generating substrate can therefore potentially be simplified.

The particulate plant material used in the aerosol-generating substrates of the present invention may be adapted to provide a desired particle size distribution. Particle size distributions herein are stated as D-values, whereby the D-value refers to the percentage of particles by number that has a diameter of less than or equal to the given D-value. For instance, in a D95 particle size distribution, 95 percent of the particles by number are of a diameter less than or equal to the given D95 value, and 5 percent of the particles by number are of a diameter measuring greater than the given D95 value. Similarly, in a D5 particle size distribution, 5 percent of the particles by number are of a diameter less than or equal to the D5 value, and 95 percent of the particles by number are of a diameter greater than the given D5 value. In combination, the D5 and D95 values therefore provide an indication of the particle size distribution of the particulate plant material.

The particulate plant material may have a D95 value of from greater than or equal to 20 microns to a D95 value of less than or equal to 300 microns. By this is meant that the particulate plant material may be of a distribution represented by any D95 value within the given range, that is D95 may be equal to 20 microns, or D95 may be equal to 25 microns, et cetera, all the way up to D95 may be equal to 300 microns. By providing a D95 value within this range, the inclusion of relatively large plant particles into the homogenised ginger material is avoided. This is desirable, since the generation of aerosol from such large plant particles is likely to be relatively inefficient. Furthermore, the inclusion of large plant particles in the homogenised ginger material may adversely impact the consistency of the material.

Preferably the particulate plant material may have a D95 value of from greater than or equal to about 50 microns to a D95 value of less than or equal to about 250 microns, more preferably a D95 value of from greater than or equal to about 100 microns to a D95 value of less than or equal to about 200 microns. The particulate ginger material and the particulate tobacco material may both have D95 values of from greater than or equal to about 20 microns to D95 values of less than or equal to about 300 microns, preferably D95 values of from greater than or equal to 50 microns to D95 values of less than or equal to about 200 microns, more preferably D95 values of from greater than or equal to about 100 microns to D95 values of less than or equal to about 200 microns.

Preferably, the particulate plant material may have a D5 value of from greater than or equal to about 10 microns to a D5 value of less than or equal to about 50 microns, more preferably a D5 value of from greater than or equal to about 15 microns to a D5 value of less than or equal to about 40 microns. By providing a D5 value within this range, the inclusion of very small dust particles into the homogenised ginger material is avoided, which may be desirable from a manufacturing point of view.

In some embodiments, the particulate plant material may be purposely ground to form particles having the desired particle size distribution. The use of purposely ground plant material advantageously improves the homogeneity of the particulate plant material and the consistency of the homogenised ginger material.

The diameter of 100 percent of the particulate plant material may be less than or equal to about 350 microns, more preferably less than or equal to about 400 microns. The diameter of 100 percent of the particulate ginger material and 100 percent of the particulate tobacco material may be

less than or equal to about 400 microns, more preferably less than or equal to about 200 microns. The particle size range of the ginger particles enables ginger particles to be combined with tobacco particles in existing cast leaf processes.

The homogenised ginger material preferably comprises at least about 55 percent by weight of the particulate plant material including ginger particles, as described above, more preferably at least about 60 percent by weight of the particulate plant material and more preferably at least about 65 percent by weight of the particulate plant material, on a dry weight basis. The homogenised ginger material preferably comprises no more than about 95 percent by weight of the particulate plant material, more preferably no more than about 90 percent by weight of the particulate plant material and more preferably no more than about 85 percent by weight of the particulate plant material, on a dry weight basis. For example, the homogenised ginger material may comprise between about 55 percent and about 95 percent by weight of the particulate plant material, or between about 60 percent and about 90 percent by weight of the particulate plant material, or between about 65 percent and about 85 percent by weight of the particulate plant material, on a dry weight basis. In one particularly preferred embodiment, the homogenised ginger material comprises about 75 percent by weight of the particulate plant material, on a dry weight basis.

The particulate plant material is therefore typically combined with one or more other components to form the homogenised ginger material.

As defined above, the homogenised ginger material further comprises a binder to alter the mechanical properties of the particulate plant material, wherein the binder is included in the homogenised ginger material during manufacturing as described herein. Suitable exogenous binders would be known to the skilled person and include but are not limited to: gums such as, for example, guar gum, xanthan gum, arabic gum and locust bean gum; cellulosic binders such as, for example, hydroxypropyl cellulose, carboxymethyl cellulose, hydroxyethyl cellulose, methyl cellulose and ethyl cellulose; polysaccharides such as, for example, starches, organic acids, such as alginic acid, conjugate base salts of organic acids, such as sodium-alginate, agar and pectins; and combinations thereof. Preferably, the binder comprises guar gum.

Preferably, the binder is present in an amount of from about 1 percent to about 10 percent by weight, based on the dry weight of the homogenised ginger material, preferably in an amount of from about 2 percent to about 5 percent by weight, based on the dry weight of the homogenised ginger material.

Alternatively or in addition, the homogenised ginger material may further comprise one or more lipids to facilitate the diffusivity of volatile components (for example, aerosol formers, gingerols and nicotine), wherein the lipid is included in the homogenised ginger material during manufacturing as described herein. Suitable lipids for inclusion in the homogenised ginger material include, but are not limited to: medium-chain triglycerides, cocoa butter, palm oil, palm kernel oil, mango oil, shea butter, soybean oil, cottonseed oil, coconut oil, hydrogenated coconut oil, candelilla wax, carnauba wax, shellac, sunflower wax, sunflower oil, rice bran, and Revel A; and combinations thereof.

Alternatively or in addition, the homogenised ginger material may further comprise a pH modifier.

Alternatively or in addition, the homogenised ginger material may further comprise fibres to alter the mechanical properties of the homogenised ginger material, wherein the

fibres are included in the homogenised ginger material during manufacturing as described herein. Suitable exogenous fibres for inclusion in the homogenised ginger material are known in the art and include fibres formed from non-tobacco material and non-ginger material, including but not limited to: cellulose fibres; soft-wood fibres; hard-wood fibres; jute fibres and combinations thereof. Exogenous fibres derived from tobacco and/or ginger can also be added. Any fibres added to the homogenised ginger material are not considered to form part of the "particulate plant material" as defined above. Prior to inclusion in the homogenised ginger material, fibres may be treated by suitable processes known in the art including, but not limited to: mechanical pulping; refining; chemical pulping; bleaching; sulfate pulping; and combinations thereof. A fibre typically has a length greater than its width.

Suitable fibres typically have lengths of greater than 400 micrometres and less than or equal to 4 mm, preferably within the range of 0.7 mm to 4 mm. Preferably, the fibres are present in an amount of at least about 2 percent by weight, based on the dry weight of the substrate. The amount of fibres in the homogenised ginger material may depend upon the type of material and in particular, the method that is used to produce the homogenised ginger material. In some embodiments, the fibres may be present in an amount of between about 2 percent by weight and about 15 percent by weight, most preferably at about 4 percent by weight, based on the dry weight of the substrate. For example, this level of fibres may be present where the homogenised ginger material is in the form of cast leaf. In other embodiments, the fibres may be present in an amount of at least about 30 percent by weight, or at least about 40 percent by weight. For example, this higher level of fibres is likely to be provided where the homogenised ginger material is a ginger paper formed in a papermaking process.

As defined above, the homogenised ginger material further comprises an aerosol former. Upon volatilisation, an aerosol former can convey other vaporised compounds released from the aerosol-generating substrate upon heating, such as nicotine and flavourants, in an aerosol. The aerosolisation of a specific compound from an aerosol-generating substrate is determined not solely by its boiling point. The quantity of a compound that is aerosolised can be affected by the physical form of the substrate, as well as by the other components that are also present in the substrate. The stability of a compound under the temperature and time frame of aerosolisation will also affect the amount of the compound that is present in an aerosol.

Suitable aerosol formers for inclusion in the homogenised ginger material are known in the art and include, but are not limited to: polyhydric alcohols, such as triethylene glycol, propylene glycol, 1,3-butanediol and glycerol; esters of polyhydric alcohols, such as glycerol mono-, di- or triacetate; and aliphatic esters of mono-, di- or polycarboxylic acids, such as dimethyl dodecanedioate and dimethyl tetradecanedioate. The homogenised ginger material may comprise a single aerosol former, or a combination of two or more aerosol formers.

The homogenised ginger material preferably has an aerosol former content of between about 5 percent and about 30 percent by weight on a dry weight basis, such as between about 10 percent and about 25 percent by weight on a dry weight basis, or between about 15 percent and about 20 percent by weight on a dry weight basis.

For example, if the substrate is intended for use in an aerosol-generating article for an electrically-operated aerosol-generating system having a heating element, it may

preferably include an aerosol former content of between about 5 percent to about 30 percent by weight on a dry weight basis. If the substrate is intended for use in an aerosol-generating article for an electrically-operated aerosol-generating system having a heating element, the aerosol former is preferably glycerol.

In other embodiments, the homogenised ginger material may have an aerosol former content of about 1 percent to about 5 percent by weight on a dry weight basis. For example, if the substrate is intended for use in an aerosol-generating article in which aerosol former is kept in a reservoir separate from the substrate, the substrate may have an aerosol former content of greater than 1 percent and less than about 5 percent. In such embodiments, the aerosol former is volatilised upon heating and a stream of the aerosol former is contacted with the aerosol-generating substrate so as to entrain the flavours from the aerosol-generating substrate in the aerosol.

The aerosol former may act as a humectant in the aerosol-generating substrate.

In preferred embodiments of the invention, the homogenised ginger material comprises ginger particles, between about 5 percent by weight and about 30 percent by weight of aerosol former and between about 1 percent by weight and about 10 percent by weight of binder, on a dry weight basis. In such embodiments, the homogenised ginger material preferably further comprises between about 2 percent by weight and about 15 percent by weight of fibers. Particularly preferably, the binder is guar gum.

Alternatively or in addition, the homogenised ginger material may further comprise an acid. The acid may comprise a carboxylic acid. The carboxylic acid may include a ketone group. Preferably the carboxylic acid may include a ketone group having less than about 10 carbon atoms, or less than about 6 carbon atoms or less than about 4 carbon atoms, such as levulinic acid or lactic acid. The inclusion of an acid may be particularly advantageous where the aerosol-generating substrate is in the form of a gel, as described below.

The homogenised plant material of the aerosol-generating substrate according to the invention may comprises a single type of homogenised plant material or two or more types of homogenised plant material having a different composition or form to each other. For example, in one embodiment, the aerosol-generating substrate comprises ginger particles and tobacco particles or cannabis particles contained within the same sheet of homogenised plant material. However, in other embodiments, the aerosol-generating substrate may comprise tobacco particles or cannabis particles and ginger particles within different sheets to each other.

The homogenised ginger material is preferably in the form of a solid or a gel. However, in some embodiments the homogenised material may be in the form of a solid that is not a gel. Preferably, the homogenised material is not in the form of a film.

The homogenised ginger material can be provided in any suitable form. For example, the homogenised ginger material may be in the form of one or more sheets. As used herein with reference to the invention, the term "sheet" describes a laminar element having a width and length substantially greater than the thickness thereof.

Alternatively or in addition, the homogenised ginger material may be in the form of a plurality of pellets or granules.

Alternatively or in addition, the homogenised ginger material may be in a form that can fill a cartridge or a shisha consumable, or that can be used in a shisha device. The

invention includes a cartridge or a shisha device that contains a homogenised ginger material.

Alternatively or in addition, the homogenised ginger material may be in the form of a plurality of strands, strips or shreds. As used herein, the term "strand" describes an elongate element of material having a length that is substantially greater than the width and thickness thereof. The term "strand" should be considered to encompass strips, shreds and any other homogenised ginger material having a similar form. The strands of homogenised ginger material may be formed from a sheet of homogenised ginger material, for example by cutting or shredding, or by other methods, for example, by an extrusion method.

In some embodiments, the strands may be formed in situ within the aerosol-generating substrate as a result of the splitting or cracking of a sheet of homogenised ginger material during formation of the aerosol-generating substrate, for example, as a result of crimping. The strands of homogenised ginger material within the aerosol-generating substrate may be separate from each other. Alternatively, each strand of homogenised ginger material within the aerosol-generating substrate may be at least partially connected to an adjacent strand or strands along the length of the strands. For example, adjacent strands may be connected by one or more fibres. This may occur, for example, where the strands have been formed due to the splitting of a sheet of homogenised ginger material during production of the aerosol-generating substrate, as described above.

Preferably, the aerosol-generating substrate is in the form of one or more sheets of homogenised ginger material. In various embodiments of the invention, the one or more sheets of homogenised ginger material may be produced by a casting process. In various embodiments of the invention, the one or more sheets of homogenised ginger material may be produced by a paper-making process. The one or more sheets as described herein may each individually have a thickness of between 100 micrometres and 600 micrometres, preferably between 150 micrometres and 300 micrometres, and most preferably between 200 micrometres and 250 micrometres. Individual thickness refers to the thickness of the individual sheet, whereas combined thickness refers to the total thickness of all sheets that make up the aerosol-generating substrate. For example, if the aerosol-generating substrate is formed from two individual sheets, then the combined thickness is the sum of the thickness of the two individual sheets or the measured thickness of the two sheets where the two sheets are stacked in the aerosol-generating substrate.

The one or more sheets as described herein may each individually have a grammage of between about 100 g/m<sup>2</sup> and about 300 g/m<sup>2</sup>.

The one or more sheets as described herein may each individually have a density of from about 0.3 g/cm<sup>3</sup> to about 1.3 g/cm<sup>3</sup>, and preferably from about 0.7 g/cm<sup>3</sup> to about 1.0 g/cm<sup>3</sup>.

The term "tensile strength" is used throughout the specification to indicate a measure of the force required to stretch a sheet of homogenised ginger material until it breaks. More specifically, the tensile strength is the maximum tensile force per unit width that the sheet material will withstand before breaking and is measured in the machine direction or cross direction of the sheet material. It is expressed in units of Newtons per meter of material (N/m). Tests for measuring the tensile strength of a sheet material are well known. A suitable test is described in the 2014 publication of the International Standard ISO 1924-2 entitled "Paper and

Board—Determination of Tensile Properties—Part 2: Constant Rate of Elongation Method".

The materials and equipment required to conduct a test according to ISO 1924-2 are: a universal tensile/compression testing machine, Instron 5566, or equivalent; a tension load cell of 100 Newtons, Instron, or equivalent; two pneumatic action grips; a steel gauge block of  $180\pm0.25$  millimetres length (width: about 10 millimetres, thickness: about 3 millimetres); a double-bladed strip cutter, size  $15\pm0.05$  about 250 millimetres, Adamel Lhomargy, or equivalent; a scalpel; a computer running acquisition software, Merlin, or equivalent; and compressed air.

The sample is prepared by first conditioning the sheet of homogenised ginger material for at least 24 hours at  $22\pm2$  degrees Celsius and  $60\pm5\%$  relative humidity before testing. A machine-direction or cross-direction sample is then cut to about  $250\times15\pm0.1$  millimetres with the double-bladed strip cutter. The edges of the test pieces must be cut cleanly, so no more than three test specimens are cut at the same time.

The tensile/compression testing instrument is set up by installing the tension load cell of 100 Newtons, switching on the Universal Tensile/Compression Testing Machine and the computer, and selecting the measurement method predefined in the software, with a test speed set to 8 millimetres per minute. The tension load cell is then calibrated and the pneumatic action grips are installed. The test distance between the pneumatic action grips is adjusted to  $180\pm0.5$  millimetres by means of the steel gauge block, and the distance and force are set to zero.

The test specimen is then placed straight and centrally between the grips, and touching the area to be tested with fingers is avoided. The upper grip is closed and the paper strip hangs in the opened lower grip. The force is set to zero. The paper strip is then pulled lightly down and the lower grip is closed; the starting force must be between 0.05 and 0.20 Newtons. While the upper grip is moving upward, a gradually increasing force is applied until the test specimen breaks. The same procedure is repeated with the remaining test specimens. The result is valid when the test specimen breaks when the grips move apart by a distance of more than 10 millimetres. If it is not the case, the result is rejected and an additional measurement is performed.

Where the test specimen of homogenised ginger material that is available is smaller than the described sample in the test according to ISO 1924-2, as set out above, the test can readily be scaled down to accommodate the available size of test specimen.

The one or more sheets of homogenised ginger material as described herein may each individually have a tensile strength at peak in a cross direction of from 50 N/m to 400 N/m or preferably from 150 N/m to 350 N/m. Given that the sheet thickness affects the tensile strength, and where a batch of sheets exhibits variation in thickness, it may be desirable to normalize the value to a specific sheet thickness.

The one or more sheets as described herein may each individually have a tensile strength at peak in a machine direction of from 100 N/m to 800 N/m or preferably from 280 N/m to 620 N/m, normalized to a sheet thickness of 215  $\mu\text{m}$ . The machine direction refers to the direction in which the sheet material would be rolled onto or unrolled from a bobbin and fed into a machine, while the cross direction is perpendicular to the machine direction. Such values of tensile strength make the sheets and methods described herein particularly suitable for subsequent operations involving mechanical stresses.

The provision of a sheet having the levels of thickness, grammage and tensile strength as defined above advanta-

geously optimises the machinability of the sheet to form the aerosol-generating substrate and ensures that damage, such as tearing of the sheet, is avoided during high speed processing of the sheet.

In embodiments of the present invention in which the aerosol-generating substrate comprises one or more sheets of homogenised ginger material, the sheets are preferably in the form of one or more gathered sheets. As used herein, the term "gathered" denotes that the sheet of homogenised ginger material is convoluted, folded, or otherwise compressed or constricted substantially transversely to the cylindrical axis of a plug or a rod. The step of "gathering" the sheet may be carried out by any suitable means which provides the necessary transverse compression of the sheet.

As used herein, the term "longitudinal" refers to the direction corresponding to the main longitudinal axis of the aerosol-generating article, which extends between the upstream and downstream ends of the aerosol-generating article. During use, air is drawn through the aerosol-generating article in the longitudinal direction. The term "transverse" refers to the direction that is perpendicular to the longitudinal axis. As used herein, the term "length" refers to the dimension of a component in the longitudinal direction and the term "width" refers to the dimension of a component in the transverse direction. For example, in the case of a plug or rod having a circular cross-section, the maximum width corresponds to the diameter of the circle.

As used herein, the term "plug" denotes a generally cylindrical element having a substantially polygonal, circular, oval or elliptical cross-section. As used herein, the term "rod" refers to a generally cylindrical element of substantially polygonal cross-section and preferably of circular, oval or elliptical cross-section. A rod may have a length greater than or equal to the length of a plug. Typically, a rod has a length that is greater than the length of a plug. A rod may comprise one or more plugs, preferably aligned longitudinally.

As used herein, the terms "upstream" and "downstream" describe the relative positions of elements, or portions of elements, of the aerosol-generating article in relation to the direction in which the aerosol is transported through the aerosol-generating article during use. The downstream end of the airflow path is the end at which aerosol is delivered to a user of the article.

The one or more sheets of homogenised ginger material may be gathered transversely relative to the longitudinal axis thereof and circumscribed with a wrapper to form a continuous rod or a plug. The continuous rod may be severed into a plurality of discrete rods or plugs. The wrapper may be a paper wrapper or a non-paper wrapper, as described in more detail below.

Alternatively, the one or more sheets of homogenised ginger material may be cut into strands as referred to above. In such embodiments, the aerosol-generating substrate comprises a plurality of strands of the homogenised ginger material. The strands may be used to form a plug. Typically, the width of such strands is at least about 0.2 mm, or at least about 0.5 mm. Preferably, the width of such strands is no more than about 5 mm, or about 4 mm, or about 3 mm, or about 1.5 mm. For example, the width of the strands may be between about 0.25 mm and about 5 mm, or between about 0.25 mm and about 3 mm, or between about 0.5 mm and about 1.5 mm.

The length of the strands is preferably greater than about 5 mm, for example, between about 5 mm to about 15 mm, or between about 8 mm to about 12 mm, or about 12 mm. Preferably, the strands have substantially the same length as

each other. The length of the strands may be determined by the manufacturing process whereby a rod is cut into shorter plugs and the length of the strands corresponds to the length of the plug. The strands may be fragile which may result in breakage especially during transit. In such cases, the length of some of the strands may be less than the length of the plug.

The plurality of strands preferably extend substantially longitudinally along the length of the aerosol-generating substrate, aligned with the longitudinal axis. Preferably, the plurality of strands are therefore aligned substantially parallel to each other. The plurality of longitudinal strands of aerosol-generating material is preferably substantially non-coiled.

The strands of homogenised ginger material preferably each have a mass to surface area ratio of at least about 0.02 milligrams per square millimetre, more preferably at least about 0.05 milligrams per square millimetre. Preferably the strands of homogenised ginger material each have a mass to surface area ratio of no more than about 0.2 milligrams per square millimetre, more preferably no more than about 0.15 milligrams per square millimetre. The mass to surface area ratio is calculated by dividing the mass of the strand of homogenised ginger material in milligrams by the geometric surface area of the strand of homogenised ginger material in square millimetres.

The one or more sheets of homogenised ginger material may be textured through crimping, embossing, or perforating. The one or more sheets may be textured prior to gathering or prior to being cut into strands. Preferably, the one or more sheets of homogenised ginger material are crimped prior to gathering, such that the homogenised ginger material may be in the form of a crimped sheet, more preferably in the form of a gathered crimped sheet. As used herein, the term "crimped sheet" denotes a sheet having a plurality of substantially parallel ridges or corrugations usually aligned with the longitudinal axis of the article.

In one embodiment, the aerosol-generating substrate may be in the form of a single plug of aerosol-generating substrate. Preferably, the plug of aerosol-generating substrate may comprise a plurality of strands of homogenised ginger material. Most preferably, the plug of aerosol-generating substrate may comprise one or more sheets of homogenised ginger material. Preferably, the one or more sheets of homogenised ginger material may be crimped such that it has a plurality of ridges or corrugations substantially parallel to the cylindrical axis of the plug. This treatment advantageously facilitates gathering of the crimped sheet of homogenised ginger material to form the plug. Preferably, the one or more sheets of homogenised ginger material may be gathered. It will be appreciated that crimped sheets of homogenised ginger material may alternatively or in addition have a plurality of substantially parallel ridges or corrugations disposed at an acute or obtuse angle to the cylindrical axis of the plug. The sheet may be crimped to such an extent that the integrity of the sheet becomes disrupted at the plurality of parallel ridges or corrugations causing separation of the material, and results in the formation of shreds, strands or strips of homogenised ginger material.

In another embodiment, the aerosol-generating substrate comprises a first plug comprising a first homogenised plant material and a second plug comprising a second homogenised plant material, wherein the first homogenised plant material and the second homogenised plant material comprise different levels of ginger particles and tobacco particles. At least one of the first homogenised plant material

and the second homogenised plant material is a homogenised ginger material. For example, the first homogenised plant material may comprise between about 50 percent and about 95 percent by weight of ginger particles on a dry weight basis; and the second homogenised plant material may comprise between about 50 percent and about 95 percent by weight of tobacco particles, on a dry weight basis. Overall, the homogenised plant materials within the aerosol-generating substrate preferably comprise at least 2.5 percent by weight of ginger particles and up to 95 percent by weight of tobacco particles, on a dry weight basis.

Optionally, the first homogenised ginger material may comprise at least 60 percent by weight of ginger particles and the second homogenised plant material may comprise at least 60 percent by weight tobacco particles. Optionally, the first homogenised ginger material may comprise at least about 90 percent by weight of ginger particles and the second homogenised ginger material may comprise at least about 90 percent by weight of tobacco particles.

In such arrangements, the first homogenised plant material preferably comprises a first particulate plant material with a higher proportion of ginger particles than the second homogenised plant material. The second homogenised plant material may be a homogenised tobacco material, with substantially no ginger particles.

Preferably, the first homogenised plant material may be in the form of one or more sheets and the second homogenised plant material may be in the form of one or more sheets.

Optionally, the aerosol-generating substrate may comprise one or more plugs. Preferably, the substrate may comprise a first plug and a second plug, wherein the first homogenised plant material may be located in the first plug and the second homogenised plant material may be located in the second plug.

Two or more plugs may be combined in an abutting end-to-end relationship and extend to form a rod. Two plugs may be placed longitudinally with a gap between them, thereby creating a cavity within a rod. The plugs may be in any suitable arrangement within the rod.

For instance, in a preferred arrangement, a downstream plug comprising a major proportion of ginger particles may abut an upstream plug comprising a major proportion of tobacco particles to form the rod. The alternative configuration in which the upstream and downstream positions of the respective plugs are changed relative to one another is also envisaged. Alternative configurations in which a third homogenised plant material containing a different proportion of ginger particles and tobacco particles and forming a third plug are also envisaged. Where two or more plugs are provided, the homogenised plant material may be provided in the same form in each plug or in a different form in each plug, that is, gathered or shredded. The one or more plugs may optionally be wrapped individually or together in a thermally conductive sheet material, as described below.

The first plug may comprise one or more sheets of the first homogenised plant material, and the second plug may comprise one or more sheets of the second homogenised plant material. The sum of the length of the plugs may be between about 10 mm and about 40 mm, preferably between about 10 and about 15 mm, more preferably about 12 mm. The first plug and the second plug may be of the same length or may have different lengths. If the first plug and the second plug have the same lengths, the length of each plug may be preferably from about 6 mm to about 20 mm. Preferably, the second plug may be longer than the first plug in order to provide a desired ratio of tobacco particles to ginger particles in the substrate. Overall, preferably the substrate

contains between 0 and 72.5 percent by weight tobacco particles and between 75 and 2.5 percent by weight ginger particles, on a dry weight basis. Preferably the second plug is at least 40 percent to 50 percent longer than the first plug.

If the first homogenised plant material and the second homogenised plant material are in the form of one or more sheets, preferably the one or more sheets of the first homogenised plant material and second homogenised plant material may be gathered sheets. Preferably the one or more sheets of the first homogenised plant material and second homogenised plant material may be crimped sheets. It will be appreciated that all other physical properties described with reference to an embodiment in which a single homogenised plant material is present are equally applicable to an embodiment in which a first homogenised plant material and a second homogenised plant material are present. Further, it will be appreciated that the description of additives (such as binders, lipids, fibres, aerosol formers, humectants, plasticisers, flavourants, fillers, aqueous and non-aqueous solvents and combinations thereof) with reference to an embodiment in which a single homogenised plant material is present are equally applicable to an embodiment in which a first homogenised plant material and a second homogenised plant material are present.

In yet another embodiment of the aerosol-generating substrate, the first homogenised plant material is in the form of a first sheet, the second homogenised plant material is in the form of a second sheet, and the second sheet at least partially overlies the first sheet.

The first sheet may be a textured sheet and the second sheet may be non-textured.

Both the first and second sheets may be textured sheets. The first sheet may be a textured sheet that is textured in a different way to the second sheet. For example, the first sheet may be crimped and the second sheet may be perforated. Alternatively, the first sheet may be perforated and the second sheet may be crimped.

Both the first and second sheets may be crimped sheets that are morphologically different from each other. For example, the second sheet may be crimped with a different number of crimps per unit width of sheet compared to the first sheet.

The sheets may be gathered to form a plug. The sheets that are gathered together to form the plug may have different physical dimensions. The width and thickness of the sheets may be varied.

It may be desirable to gather together two sheets each having a different thickness or each having a different width. This may alter the physical properties of the plug. This may facilitate the formation of a blended plug of aerosol-generating substrate from sheets of different chemical composition.

The first sheet may have a first thickness and the second sheet may have a second thickness that is a multiple of the first thickness, for example the second sheet may have a thickness two or three times the first thickness.

The first sheet may have a first width and the second sheet may have a second width that is different to the first width.

The first sheet and the second sheet may be disposed in overlapping relationship prior to being gathered together, or at the point at which they are gathered together. The sheets may have the same width and thickness. The sheets may have different thicknesses. The sheets may have different widths. The sheets may be differently textured.

Where it is desired that the first sheet and the second sheet are both textured, the sheets may be simultaneously textured prior to being gathered. For example, the sheets may be

brought into overlapping relationship and passed through a texturing means, such as a pair of crimping rollers. A suitable apparatus and process for simultaneous crimping are described with reference to FIG. 2 of WO-A-2013/178766. In a preferred embodiment, the second sheet of the second homogenised plant material overlies the first sheet of the first homogenised plant material, and the combined sheets are gathered to form a plug of aerosol-generating substrate. Optionally, the sheets may be crimped together prior to gathering to facilitate gathering.

Alternatively, each sheet may be separately textured and then subsequently brought together to be gathered into a plug. For example, where the two sheets have a different thickness, it may be desirable to crimp the first sheet differently relative to the second sheet.

It will be appreciated that all other physical properties described with reference to an embodiment in which a single homogenised ginger material is present are equally applicable to an embodiment in which a first homogenised plant material and a second homogenised plant material are present. Further, it will be appreciated that the description of additives (such as binders, lipids, fibres, aerosol formers, humectants, plasticisers, flavourants, fillers, aqueous and non-aqueous solvents and combinations thereof) with reference to an embodiment in which a single homogenised ginger material is present are equally applicable to an embodiment in which a first homogenised plant material and a second homogenised plant material are present.

The homogenised ginger material used in the aerosol-generating substrates according to the invention may be produced by various methods including paper making, casting, dough reconstitution, extrusion or any other suitable process.

Preferably, the homogenised ginger material is in the form of "cast leaf". The term "cast leaf" is used herein to refer to a sheet product made by a casting process that is based on casting a slurry comprising plant particles (for example, ginger particles, or tobacco particles and ginger particles in a mixture) and a binder (for example, guar gum) onto a supportive surface, such as a belt conveyor, drying the slurry and removing the dried sheet from the supportive surface. An example of the casting or cast leaf process is described in, for example, U.S. Pat. No. 5,724,998 for making cast leaf tobacco. In a cast leaf process, particulate plant materials are mixed with a liquid component, typically water, to form a slurry. Other added components in the slurry may include fibres, a binder and an aerosol former. The particulate plant materials may be agglomerated in the presence of the binder. The slurry is cast onto a supportive surface and dried to form a sheet of homogenised ginger material.

In certain preferred embodiments, the homogenised ginger material used in articles according to the present invention is produced by casting. Homogenised ginger material made by the casting process typically comprise agglomerated particulate plant material.

In a cast-leaf process, because substantially all the soluble fraction is kept within the plant material, most flavours are advantageously preserved. Additionally, energy-intensive paper-making steps are avoided.

In one preferred embodiment of the present invention, to form homogenised ginger material, a mixture comprising particulate plant material, water, a binder, and an aerosol former is formed. A sheet is formed from the mixture, and the sheet is then dried. Preferably the mixture is an aqueous mixture. As used herein, "dry weight" refers to the weight of a particular non-water component relative to the sum of the weights of all non-water components in a mixture, expressed

as a percentage. The composition of aqueous mixtures may be referred to by "percentage dry weight." This refers to the weight of the non-water components relative to the weight of the entire aqueous mixture, expressed as a percentage.

The mixture may be a slurry. As used herein, a "slurry" is a homogenised aqueous mixture with a relatively low dry weight. A slurry as used in the method herein may preferably have a dry weight of between 5 percent and 60 percent.

Alternatively, the mixture may be a dough. As used herein, a "dough" is an aqueous mixture with a relatively high dry weight. A dough as used in the method herein may preferably have a dry weight of at least 60 percent, more preferably at least 70 percent.

Slurries comprising greater than 30 percent dry weight and doughs may be preferred in certain embodiments of the present method.

The step of mixing the particulate plant material, water and other optional components may be carried out by any suitable means. For mixtures of a low viscosity, that is, some slurries, it is preferred that mixing is performed using a high energy mixer or a high shear mixer. Such mixing breaks down and distributes the various phases of the mixture homogeneously. For mixtures of a higher viscosity, that is, some doughs, a kneading process may be used to distribute the various phases of the mixture homogeneously.

Methods according to the present invention may further comprise the step of vibrating the mixture to distribute the various components. Vibrating the mixture, that is for example vibrating a tank or silo where a homogenised mixture is present, may help the homogenization of the mixture, particularly when the mixture is a mixture of low viscosity, that is, some slurries. Less mixing time may be required to homogenize a mixture to the target value optimal for casting if vibrating is performed as well as mixing.

If the mixture is a slurry, a web of homogenised ginger material is preferably formed by a casting process comprising casting the slurry on a supportive surface, such as a belt conveyor. The method for production of a homogenised ginger material comprises the step of drying said cast web to form a sheet. The cast web may be dried at room temperature or at an ambient temperature of at least about 60 degrees Celsius, more preferably at least about 80 degrees Celsius for a suitable length of time. Preferably, the cast web is dried at an ambient temperature of no more than 200 degrees Celsius, more preferably no more than about 160 degrees Celsius. For example, the cast web may be dried at a temperature of between about 60 degrees Celsius and about 200 degrees Celsius, or between about 80 degrees Celsius and about 160 degrees Celsius. Preferably, the moisture content of the sheet after drying is between about 5 percent and about 15 percent based on the total weight of the sheet. The sheet may then be removed from the supportive surface after drying. The cast sheet has a tensile strength such that it can be mechanically manipulated and wound or unwound from a bobbin without breakage or deformation.

If the mixture is a dough, the dough may be extruded in the form of a sheet, strands, or strips, prior to the step of drying the extruded mixture. Preferably, the dough may be extruded in the form of a sheet. The extruded mixture may be dried at room temperature or at a temperature of at least about 60 degrees Celsius, more preferably at least about 80 degrees Celsius for a suitable length of time. Preferably, the cast web is dried at an ambient temperature of no more than 200 degrees Celsius, more preferably no more than about 160 degrees Celsius. For example, the cast web may be dried at a temperature of between about 60 degrees Celsius and about 200 degrees Celsius, or between about 80 degrees

Celsius and about 160 degrees Celsius. Preferably, the moisture content of the extruded mixture after drying is between about 5 percent and about 15 percent based on the total weight of the sheet. A sheet formed from dough requires less drying time and/or lower drying temperatures as a result of significantly lower water content relative to a web formed from a slurry.

After the sheet has been dried, the method may optionally comprise a step of coating a nicotine salt, preferably along with an aerosol former, onto the sheet, as described in the disclosure of WO-A-2015/082652.

After the sheet has been dried, methods according to the invention may optionally comprise a step of cutting the sheet into strands, shreds or strips for the formation of the aerosol-generating substrate as described above. The strands, shreds or strips may be brought together to form a rod of the aerosol-generating substrate using suitable means. In the formed rod of aerosol-generating substrate, the strands, shreds or strips may be substantially aligned, for example, in the longitudinal direction of the rod. Alternatively, the strands, shreds or strips may be randomly oriented in the rod.

Methods according to the present invention may optionally further comprise a step of winding the sheet onto a bobbin, after the drying step.

The present invention further provides an alternative paper-making method for producing sheets of homogenised ginger material in the form of "plant paper".

Plant paper refers to a reconstituted plant sheet formed by a process in which a plant feedstock is extracted with a solvent to produce an extract of soluble plant compounds and an insoluble residue of fibrous plant material, and the extract is recombined with the insoluble residue. The extract may optionally be concentrated or further processed before being recombined with the insoluble residue. The insoluble residue may optionally be refined and combined with additional plant fibers before being recombined with the extract. In the method according to the present invention, the plant feedstock will comprise particles of ginger, optionally in combination with particles of tobacco.

In more detail, the method of producing a plant paper comprises a first step of mixing a plant material and water to form a dilute suspension. The dilute suspension comprises mostly separate cellulose fibres. The suspension has a lower viscosity and a higher water content than the slurry produced in the casting process. This first step may involve soaking, optionally in the presence of an alkali, such as sodium hydroxide, and optionally applying heat.

The method further comprises a second step of separating the suspension into an insoluble portion containing the insoluble residue of fibrous plant material and a liquid or aqueous extract comprising soluble plant compounds. The water remaining in the insoluble residue of fibrous plant material may be drained through a screen, acting as a sieve, such that a web of randomly interwoven fibres may be laid down. Water may be further removed from this web by pressing with rollers, sometimes aided by suction or vacuum.

After removal of the aqueous portion and water, the insoluble residue is formed into a sheet. Preferably, a generally flat, uniform sheet of plant fibres is formed.

Preferably, the method further comprises the steps of concentrating the extract of soluble plant compounds that were removed from the sheet and adding the concentrated extract into the sheet of insoluble fibrous plant material to form a sheet of homogenised ginger material. Alternatively or in addition, a soluble plant substance or concentrated plant substance from another process can be added to the

sheet. The extract or concentrated extract may be from another variety of the same species of plant, or from another species of plant.

This process, as described in U.S. Pat. No. 3,860,012, has been used with tobacco to make reconstituted tobacco products, also known as tobacco paper. The same process can also be used with one or more plants to produce a paper-like sheet material, such a sheet of ginger paper.

In certain preferred embodiments, the homogenised ginger material used in articles according to the present invention is produced by a paper-making process as defined above. In such embodiments, the homogenised ginger material is in the form of a ginger paper.

Homogenised tobacco material or homogenised ginger material produced by such a process are referred to as tobacco paper or ginger paper. Homogenised plant material made by the paper-making process is distinguishable by the presence of a plurality of fibres throughout the material, visible by eye or under a light microscope, particularly when the paper is wetted by water. In contrast, homogenised plant material made by the casting process comprises less fibres than paper and tends to dissociate into a slurry when it is wetted. Mixed tobacco ginger paper refers to homogenised plant material produced by such a process using a mixture of tobacco and ginger materials.

In embodiments in which the aerosol-generating substrate comprises a combination of ginger particles and tobacco particles, the aerosol-generating substrate may comprise one or more sheets of ginger paper and one or more sheets of tobacco paper. The sheets of ginger paper and tobacco paper may be interleaved with each other or stacked prior to being gathered to form a rod. Optionally, the sheets may be crimped. Alternatively, the sheets of ginger paper and tobacco paper may be cut into strands, strips or shreds and then combined to form a rod. The relative amounts of tobacco and ginger in the aerosol-generating substrate can be adjusted by changing the respective number of tobacco and ginger sheets or the respective amounts of ginger and tobacco strands, strips or shreds in the rod.

For example, the number or amount of tobacco and ginger sheets or strands may be adjusted to provide a ratio of ginger to tobacco of about 1:4, or about 1:9 or about 1:30.

Other known processes that can be applied to producing homogenised plant materials are dough reconstitution processes of the type described in, for example, U.S. Pat. No. 3,894,544; and extrusion processes of the type described in, for example, in GB-A-983,928. Typically, the densities of homogenised plant materials produced by extrusion processes and dough reconstitution processes are greater than the densities of the homogenised plant materials produced by casting processes.

In alternative embodiments of the present invention, the homogenised ginger material is in the form of a gel composition formed with the ginger particles, aerosol former and binder.

Preferably, where the homogenised ginger material is in the form of a gel composition containing the ginger particles, the binder comprises a cellulose ether such as carboxymethyl cellulose. The binder may be present in an amount of between about 1 percent and about 5 percent by weight, based on the total weight of the gel. For example, the gel composition may comprise between 1.5 percent by weight and 3.5 percent by weight of sodium carboxymethyl cellulose.

Preferably, the gel composition comprises at least about 60 percent by weight of aerosol former, such as glycerin, based on the total weight of the gel. For example, the gel

composition may comprise between 65 percent by weight and 85 percent by weight of glycerin.

Optionally, the gel composition may further comprise an acid, such as lactic acid. The acid may be present in an amount of up to about 6 percent by weight, based on the total weight of the gel composition. Optionally, the gel composition may comprise up to about 5 percent by weight of nicotine, based on the total weight of the gel composition. Optionally, the gel composition comprises between about 10 percent by weight and about 30 percent by weight of water, based on the total weight of the gel composition.

In embodiments in which the homogenised ginger material is in the form of a gel composition, the aerosol-generating substrate preferably comprises a porous medium loaded with the gel composition. The term "porous" is used herein to refer to a material that provides a plurality of pores or openings that allow the passage of air through the material.

The porous medium may be any suitable porous material able to hold or retain the gel composition. Ideally the porous medium can allow the gel composition to move within it. In specific embodiments the porous medium comprises natural materials, synthetic, or semi-synthetic, or a combination thereof. In specific embodiments the porous medium comprises sheet material, foam, or fibers, for example loose fibers; or a combination thereof. In specific embodiments the porous medium comprises a woven, non-woven, or extruded material, or combinations thereof. Preferably the porous medium comprises, cotton, paper, viscose, PLA, or cellulose acetate, of combinations thereof. Preferably the porous medium comprises a sheet material, for example, cotton or cellulose acetate. In a particularly preferred embodiment, the porous medium comprises a sheet made from cotton fibers.

The porous medium used in the present invention may be crimped or shredded. In preferred embodiments, the porous medium is crimped. In alternative embodiments the porous medium comprises shredded porous medium. The crimping or shredding process can be before or after loading with the gel composition.

Preferably, when the homogenised ginger material is in the form of a gel composition loaded onto a porous medium, the aerosol-generating substrate comprises an elongate susceptor element extending longitudinally through the porous medium or adjacent to the porous medium.

Preferably, the aerosol-generating substrate of aerosol-generating articles according to the invention comprises at least about 200 mg of the homogenised plant material, more preferably at least about 250 mg of the homogenised plant material and more preferably at least about 300 mg of the homogenised plant material.

Aerosol-generating articles according to the invention comprise a rod, comprising the aerosol-generating substrate in one or more plugs. The rod of aerosol-generating substrate may have a length of from about 5 mm to about 120 mm. For example, the rod may preferably have a length of between about 10 and about 45 mm, more preferably between about 10 mm and 15 mm, most preferably about 12 mm.

In alternative embodiments, the rod preferably has a length of between about 30 mm and about 45 mm, or between about 33 mm and about 41 mm. Where the rod is formed of a single plug of aerosol-generating substrate, the plug has the same length as the rod.

The rod of aerosol-generating substrate may have an external diameter of between about 5 mm and about 10 mm, depending on their intended use. For example, in some embodiments, the rod may have an external diameter of

between about 5.5 mm and about 8 mm, or between about 6.5 mm and about 8 mm. The "external diameter of the rod of aerosol-generating substrate corresponds to the diameter of the rod including any wrappers.

The rod of aerosol-generating substrate of the aerosol-generating articles according to the invention is preferably circumscribed by one or more wrappers along at least a part of its length. The one or more wrappers may include a paper wrapper or a non-paper wrapper, or both. Suitable paper wrappers for use in specific embodiments of the invention are known in the art and include, but are not limited to: cigarette papers; and filter plug wraps. Suitable non-paper wrappers for use in specific embodiments of the invention are known in the art and include, but are not limited to sheets of homogenised tobacco materials. Homogenised tobacco wrappers are particularly suitable for use in embodiments wherein the aerosol-generating substrate comprises one or more sheets of homogenised ginger material formed of particulate plant material, the particulate plant material containing ginger particles in combination with a low percentage by weight of tobacco particles, such as from 20 percent to 0 percent by weight of tobacco particles, based on dry weight.

In certain embodiments of the invention, the aerosol-generating substrate is circumscribed along at least a part of its length by a thermally conductive sheet material, for example, a metallic foil, such as aluminium foil or a metallised paper. The metallic foil or metallised paper serves the purpose of conducting heat rapidly throughout the aerosol-generating substrate. In addition, the metallic foil or metallised paper may serve to prevent the ignition of the aerosol-generating substrate in the event that the consumer attempts to light it. Furthermore, during use, the metallic foil or metallised paper may prevent odours produced upon heating of the outer wrapper from entering the aerosol generated from the aerosol-generating substrate. For example, this may be a problem for aerosol-generating articles having an aerosol-generating substrate that is heated externally during use in order to generate an aerosol. Alternatively, or in addition, a metallised wrapper may be used to facilitate detection or recognition of the aerosol-generating article when it is inserted into an aerosol-generating device during use. The metallic foil or metallised paper may comprise metal particles, such as iron particles.

The one or more wrappers circumscribing the aerosol-generating substrate preferably have a total thickness of between about 0.1 mm and about 0.9 mm.

The internal diameter of the rod of aerosol-generating substrate is preferably between about 3 mm and about 9.5 mm, more preferably between about 4 mm and about 7.5 mm, more preferably between about 5 mm and about 7.5 mm. The "internal diameter" corresponds to the diameter of the rod of aerosol-generating substrate without including the thickness of the wrappers, but measured with the wrappers still in place.

Aerosol-generating articles according to the invention also include but are not limited to a cartridge or a shisha consumable.

Aerosol-generating articles according to the invention may optionally include a support element comprising at least one hollow tube immediately downstream of the aerosol-generating substrate. One function of the tube is to locate the aerosol-generating substrate towards the distal end of the aerosol-generating article so that it can be contacted with a heating element. The tube acts to prevent the aerosol-generating substrate from being forced along the aerosol-generating article towards other downstream elements when

a heating element is inserted into the aerosol-generating substrate. The tube also acts as a spacer element to separate the downstream elements from the aerosol-generating substrate. The tube can be made of any material, such as cellulose acetate, a polymer, cardboard, or paper.

Alternatively or in addition to a support element, aerosol-generating articles according to the invention may optionally comprise an aerosol-cooling element downstream of the aerosol-generating substrate and immediately downstream of the hollow tube forming the support element. In use, an aerosol formed by volatile compounds released from the aerosol-generating substrate passes through and is cooled by the aerosol-cooling element before being inhaled by a user. The lower temperature allows the vapours to condense into an aerosol. The aerosol-cooling element may be a hollow tube, such as a hollow cellulose acetate tube or a cardboard tube, which can be similar to the support element that is immediately downstream of the aerosol-generating substrate. The aerosol cooling element may be a hollow tube of equal outer diameter but smaller or larger inner diameter than the hollow tube of the support element.

In one embodiment, the aerosol-cooling element wrapped in paper comprises one or more longitudinal channels made of any suitable material, such as a metallic foil, a paper laminated with a foil, a polymeric sheet preferably made of a synthetic polymer, and a substantially non-porous paper or cardboard. In some embodiments, the aerosol-cooling element wrapped in paper may comprise one or more sheets made of a material selected from the group consisting of polyethylene (PE), polypropylene (PP), polyvinylchloride (PVC), polyethylene terephthalate (PET), polylactic acid (PLA), cellulose acetate (CA), paper laminated with a polymeric sheet and aluminium foil. Alternatively, the aerosol-cooling element may be made of woven or non-woven filaments of a material selected from the group consisting of polyethylene (PE), polypropylene (PP), polyvinylchloride (PVC), polyethylene terephthalate (PET), polylactic acid (PLA), and cellulose acetate (CA). In a preferred embodiment, the aerosol-cooling element is a crimped and gathered sheet of polylactic acid wrapped within a filter paper. In another preferred embodiment, the aerosol-cooling element comprises a longitudinal channel and is made of woven filaments of a synthetic polymer, such as polylactic acid filaments, which are wrapped in paper.

One or more additional hollow tubes may be provided downstream of the aerosol-cooling element.

Aerosol-generating articles according to the invention may further comprise a filter or mouthpiece downstream of the aerosol-generating substrate and, where present, the support element and aerosol-cooling element. The filter may comprise one or more filtration materials for the removal of particulate components, gaseous components, or a combination thereof. Suitable filtration materials are known in the art and include, but are not limited to: fibrous filtration materials such as, for example, cellulose acetate tow and paper; adsorbents such as, for example, activated alumina, zeolites, molecular sieves and silica gel; biodegradable polymers including, for example, polylactic acid (PLA), Mater-Bi®, hydrophobic viscose fibres, and bioplastics; and combinations thereof. The filter may be located at the downstream end of the aerosol-generating article. The filter may be a cellulose acetate filter plug. The filter is about 7 mm in length in one embodiment, but may have a length of between about 5 mm and about 10 mm. Aerosol-generating articles according to the invention may comprise a mouth end cavity at the downstream end of the article. The mouth end cavity may be defined by one or more wrappers extend-

ing downstream from the filter or mouthpiece. Alternatively, the mouth end cavity may be defined by a separate tubular element provided at the downstream end of the aerosol-generating article.

Aerosol-generating articles according to the invention preferably further comprise a ventilation zone provided at a location along the aerosol-generating article. For example, the aerosol-generating article may be provided at a location along a hollow tube provided downstream of the aerosol-generating substrate.

Aerosol-generating articles according to the invention may optionally further comprise an upstream element at the upstream end of the aerosol-generating substrate. The upstream element may be a porous plug element, such as a plug of fibrous filtration material such as cellulose acetate.

In preferred embodiments of the invention, the aerosol-generating article comprises the aerosol-generating substrate, at least one hollow tube downstream of the aerosol-generating substrate and a filter downstream of the at least one hollow tube. Optionally, the aerosol-generating article further comprises a mouth end cavity at the downstream end of the filter. Optionally, the aerosol-generating article further comprises an upstream element at the upstream end of the aerosol-generating substrate. Preferably, a ventilation zone is provided at a location along the at least one hollow tube.

In a particularly preferred embodiment having this arrangement, the aerosol-generating article comprises an aerosol-generating substrate, an upstream element at the upstream end of the aerosol-generating substrate, a support element downstream of the aerosol-generating substrate, an aerosol-cooling element downstream of the support element and a filter downstream of the aerosol-cooling element. Preferably, the support element and the aerosol-cooling element are both in the form of a hollow tube. Preferably, the aerosol-generating substrate comprises an elongate susceptor element extending longitudinally through it.

In one particularly preferred example, the aerosol-generating substrate has a length of about 33 mm and an external diameter of between about 5.5 mm and 6.7 mm, wherein the aerosol-generating substrate comprises about 340 mg of the homogenised ginger material in the form of a plurality of strands, wherein the homogenised ginger material comprises about 14 percent by weight glycerol on a dry weight basis. In this embodiment, the aerosol-generating article has a total length of about 74 mm and comprises a cellulose acetate tow filter having a length of about 10 mm, as well as a mouth end cavity defined by a hollow tube having a length of about 6-7 mm. The aerosol-generating article comprises a hollow tube downstream of the aerosol-generating substrate, wherein the hollow tube has a length of about 25 mm and is provided with a ventilation zone.

The aerosol-generating articles according to the invention may have a total length of at least about 30 mm, or at least about 40 mm. The total length of the aerosol-generating article may be less than 90 mm, or less than about 80 mm.

In one embodiment, the aerosol-generating article has a total length of between about 40 mm and about 50 mm, preferably about 45 mm. In another embodiment, the aerosol-generating article has a total length of between about 70 mm and about 90 mm, preferably between about 80 mm and about 85 mm. In another embodiment, the aerosol-generating article has a total length of between about 72 mm and about 76 mm, preferably about 74 mm.

The aerosol-generating article may have an external diameter of about 5 mm to about 8 mm, preferably between about 6 mm and about 8 mm. In one embodiment, the aerosol-generating article has an external diameter of about 7.3 mm.

Aerosol-generating articles according to the invention may further comprise one or more aerosol-modifying elements. An aerosol-modifying element may provide an aerosol-modifying agent. As used herein, the term aerosol-modifying agent is used to describe any agent that, in use, modifies one or more features or properties of aerosol passing through the filter. Suitable aerosol-modifying agents include, but are not limited to, agents that, in use, impart a taste or aroma to aerosol passing through the filter, or agents that, in use, remove flavors from the aerosol passing through the filter.

An aerosol-modifying agent may be one or more of moisture or a liquid flavourant. Water or moisture may modify the sensorial experience of the user, for example by moistening the generated aerosol, which may provide a cooling effect on the aerosol and may reduce the perception of harshness experienced by the user. An aerosol-modifying element may be in the form of a flavour-delivery element to deliver one or more liquid flavourants. Alternatively, a liquid flavorant may be added directly to the homogenised ginger material, for example, by adding the flavour to the slurry or feedstock during production of the homogenised ginger material, or by spraying the liquid flavourant onto the surface of the homogenised ginger material.

The one or more liquid flavourants may comprise any flavour compound or botanical extract suitable for being releasably disposed in liquid form within the flavour-delivery element to enhance the taste of aerosol produced during use of the aerosol-generating article. The flavourants, liquid or solid, can also be disposed directly in the material which forms the filter, such as cellulose acetate tow. Suitable flavours or flavourings include, but are not limited to, menthol, mint, such as peppermint and spearmint, chocolate, liquorice, citrus and other fruit flavours, gamma octalactone, vanillin, ethyl vanillin, breath freshener flavours, spice flavours such as cinnamon, methyl salicylate, linalool, eugenol, bergamot oil, geranium oil, lemon oil, cannabis oil, and tobacco flavour. Other suitable flavours may include flavour compounds selected from the group consisting of an acid, an alcohol, an ester, an aldehyde, a ketone, a pyrazine, combinations or blends thereof and the like.

In certain embodiments of the invention, the aerosol-modifying agent may be an essential oil derived from one or more plants. For example, the homogenised ginger material may comprise a ginger oil, such as ginger essential oil, to further enhance the ginger flavours delivered to the consumer upon heating.

In certain embodiments of the invention, the aerosol-generating substrate may comprise a homogenised plant material comprising particulate plant material, such as tea particles, in combination with ginger oil.

An aerosol-modifying agent may be an adsorbent material such as activated carbon, which removes certain constituents of the aerosol passing through the filter and thereby modifies the flavour and aroma of the aerosol.

The one or more aerosol-modifying elements may be located downstream of the aerosol-generating substrate or within the aerosol-generating substrate. The aerosol-generating substrate may comprise homogenised ginger material and an aerosol-modifying element. In various embodiments, the aerosol-modifying element may be placed adjacent to the homogenised ginger material or embedded in the homogenised ginger material. Typically, aerosol-modifying elements may be located downstream of the aerosol-generating substrate, most typically, within the aerosol-cooling element, within the filter of the aerosol-generating article, such as within a filter plug or within a cavity, preferably within a

cavity between filter plugs. The one or more aerosol-modifying elements may be in the form of one or more of a thread, a capsule, a microcapsule, a bead or a polymer matrix material, or a combination thereof.

If an aerosol-modifying element is in the form of a thread, as described in WO-A-2011/060961, the thread may be formed from paper such as filter plug wrap, and the thread may be loaded with at least one aerosol-modifying agent and located within the body of the filter. Other materials that can be used to form a thread include cellulose acetate and cotton.

If an aerosol-modifying element is in the form of a capsule, as described in WO-A-2007/010407, WO-A-2013/068100 and WO-A-2014/154887, the capsule may be a breakable capsule located within the filter, the inner core of the capsule containing an aerosol-modifying agent which may be released upon breakage of the outer shell of the capsule when the filter is subjected to external force. The capsule may be located within a filter plug or within a cavity, or within a cavity between filter plugs.

If an aerosol-modifying element is in the form of a polymer matrix material, the polymer matrix material releases the flavourant when the aerosol-generating article is heated, such as when the polymer matrix is heated above the melting point of the polymer matrix material as described in WO-A-2013/034488. Typically, such polymer matrix material may be located within a bead within the aerosol-generating substrate. Alternatively, or in addition, the flavourant may be trapped within the domains of a polymer matrix material and releasable from the polymer matrix material upon compression of the polymer matrix material. Preferably, the flavorant is released upon compression of the polymer matrix material with a force of around 15 Newtons. Such flavour-modifying elements may provide a sustained release of the liquid flavourant over a range of force of at least 5 Newtons, such as between 5N and 20N, as described in WO-A-2013/068304. Typically, such polymer matrix material may be located within a bead within the filter.

The aerosol-generating article may comprise a combustible heat source and an aerosol-generating substrate downstream of the combustible heat source, the aerosol-generating substrate as described above with respect to the first aspect of the invention.

For example, substrates as described herein may be used in heated aerosol-generating articles of the type disclosed in WO-A-2009/022232, which comprise a combustible carbon-based heat source, an aerosol-generating substrate downstream of the combustible heat source, and a heat-conducting element around and in contact with a rear portion of the combustible carbon-based heat source and an adjacent front portion of the aerosol-generating substrate. However, it will be appreciated that substrates as described herein may also be used in heated aerosol-generating articles comprising combustible heat sources having other constructions.

The present invention provides an aerosol-generating system comprising an aerosol-generating device comprising a heating element, and an aerosol-generating article for use with the aerosol-generating device, the aerosol-generating article comprising the aerosol-generating substrate as described above.

In a preferred embodiment, aerosol-generating substrates as described herein may be used in heated aerosol-generating articles for use in electrically-operated aerosol-generating systems in which the aerosol-generating substrate of the heated aerosol-generating article is heated by an electrical heat source.

For example, aerosol-generating substrates as described herein may be used in heated aerosol-generating articles of the type disclosed in EP-A-0 822 760.

The heating element of such aerosol-generating devices may be of any suitable form to conduct heat. The heating of the aerosol-generating substrate may be achieved internally, externally or both. The heating element may preferably be a heater blade or pin adapted to be inserted into the substrate so that the substrate is heated from inside. Alternatively, the heating element may partially or completely surround the substrate and heat the substrate circumferentially from the outside.

The aerosol-generating system may be an electrically-operated aerosol generating system comprising an inductive heating device. Inductive heating devices typically comprise an induction source that is configured to be coupled to a susceptor, which may be provided externally to the aerosol-generating substrate or internally within the aerosol-generating substrate. The induction source generates an alternating electromagnetic field that induces magnetization or eddy currents in the susceptor. The susceptor may be heated as a result of hysteresis losses or induced eddy currents which heat the susceptor through ohmic or resistive heating.

Electrically operated aerosol-generating systems comprising an inductive heating device may also comprise the aerosol-generating article having the aerosol-generating substrate and a susceptor in thermal proximity to the aerosol-generating substrate. Typically, the susceptor is in direct contact with the aerosol-generating substrate and heat is transferred from the susceptor to the aerosol-generating substrate primarily by conduction. Examples of electrically operated aerosol-generating systems having inductive heating devices and aerosol-generating articles having susceptors are described in WO-A1-95/27411 and WO-A1-2015/177255.

A susceptor may be a plurality of susceptor particles which may be deposited on or embedded within the aerosol-generating substrate. When the aerosol-generating substrate is in the form of one or more sheets, a plurality of susceptor particles may be deposited on or embedded within the one or more sheets. The susceptor particles are immobilized by the substrate, for example, in sheet form, and remain at an initial position. Preferably, the susceptor particles may be homogeneously distributed in the homogenised ginger material of the aerosol-generating substrate. Due to the particulate nature of the susceptor, heat is produced according to the distribution of the particles in the homogenised ginger material sheet of the substrate. Alternatively, the susceptor in the form of one or more sheets, strips, shreds or rods may also be placed next to the homogenised ginger material or used as embedded in the homogenised ginger material. In one embodiment, the aerosol forming substrate comprises one or more susceptor strips. For example, the rod of aerosol-generating substrate may comprise an elongate susceptor element extending longitudinally through it. In another embodiment, the susceptor is present in the aerosol-generating device.

The susceptor may have a heat loss of more than 0.05 Joule per kilogram, preferably a heat loss of more than 0.1 Joule per kilogram. Heat loss is the capacity of the susceptor to transfer heat to the surrounding material. Because the susceptor particles are preferably homogeneously distributed in the aerosol-generating substrate, a uniform heat loss from the susceptor particles may be achieved thus generating a uniform heat distribution in the aerosol-generating substrate and leading to a uniform temperature distribution in the aerosol-generating article. It has been found that a

specific minimal heat loss of 0.05 Joule per kilogram in the susceptor particles allows for heating of the aerosol-generating substrate to a substantially uniform temperature, thus providing aerosol generation. Preferably, the average temperatures achieved within the aerosol-generating substrate in such embodiments are about 200 degree Celsius to about 240 degrees Celsius.

Reducing the risk of overheating the aerosol-generating substrate may be supported by the use of susceptor materials having a Curie temperature, which allows a heating process due to hysteresis loss only up to a certain maximum temperature. The susceptor may have a Curie temperature between about 200 degree Celsius and about 450 degree Celsius, preferably between about 240 degree Celsius and about 400 degree Celsius, for example about 280 degree Celsius. When a susceptor material reaches its Curie temperature, the magnetic properties change. At the Curie temperature the susceptor material changes from a ferromagnetic phase to a paramagnetic phase. At this point, heating based on energy loss due to orientation of ferromagnetic domains stops. Further heating is then mainly based on eddy current formation such that a heating process is automatically reduced upon reaching the Curie temperature of the susceptor material. Preferably, susceptor material and its Curie temperature are adapted to the composition of the aerosol-generating substrate in order to achieve an optimal temperature and temperature distribution in the aerosol-generating substrate for an optimum aerosol generation.

In some preferred embodiments of the aerosol-generating article according to the invention, the susceptor is made of ferrite. Ferrite is a ferromagnet with a high magnetic permeability and especially suitable as susceptor material. The main component of ferrite is iron. Other metallic components, for example, zinc, nickel, manganese, or non-metallic components, for example silicon, may be present in varying amounts. Ferrite is a relatively inexpensive, commercially available material. Ferrite is available in particle form in the size ranges of the particles used in the particulate plant material forming the homogenised ginger material according to the invention. Preferably, the particles are a fully sintered ferrite powder, such as for example FP160, FP215, FP350 by PPT, Indiana USA.

In certain embodiments of the invention, the aerosol-generating system comprises an aerosol-generating article comprising an aerosol-generating substrate as defined above, a source of aerosol former and a means to vaporise the aerosol former, preferably a heating element as described above. The source of aerosol former can be a reservoir, which can be refillable or replaceable, that resides on the aerosol generating device. While the reservoir is physically separate from the aerosol generating article, the vapour that is generated is directed through the aerosol-generating article. The vapour makes contact with the aerosol-generating substrate which releases volatile compounds, such as nicotine and flavourants in the particulate plant material, to form an aerosol. Optionally, to aid volatilization of compounds in the aerosol-generating substrate, the aerosol-generating system may further comprise a heating element to heat the aerosol-generating substrate, preferably in a co-ordinated manner with the aerosol former. However, in certain embodiments, the heating element used to heat the aerosol generating article is separate from the heater that heats the aerosol former.

As defined above, the present invention further provides an aerosol produced upon heating of an aerosol-generating substrate, wherein the aerosol comprises specific amounts

and ratios of the characteristic compounds derived from ginger particles as defined above.

According to the invention, the aerosol comprises [6]-gingerol in an amount of at least 0.3 micrograms per puff of aerosol; [10]-gingerol in an amount of at least 0.03 micrograms per puff of aerosol; [10]-shogaol in an amount of at least 0.7 micrograms per puff or aerosol, [8]-shogaol in an amount of at least 0.3 micrograms per puff of aerosol and [6]-shogaol in an amount of at least 0.6 micrograms per puff of aerosol. For the purposes of the present invention, a "puff" is defined as a volume of aerosol released from an aerosol-generating substrate upon heating and collected for analysis, wherein the puff of aerosol has a puff volume of 55 millilitres as generated by a smoking machine. Accordingly, any reference herein to a "puff" of aerosol should be understood to refer to a 55 millilitre puff unless stated otherwise.

The ranges indicated define the total amount of each component measured in a 55 millilitre puff of aerosol. The aerosol may be generated from an aerosol-generating substrate using any suitable means and may be trapped and analysed as described above in order to identify the characteristic compounds within the aerosol and measure the amounts thereof. For example, the "puff" may correspond to a 55 millilitre puff taken on a smoking machine such as that used in the Health Canada test method described herein.

Preferably, the aerosol according to the present invention comprises at least about 5 micrograms of [6]-gingerol per puff of aerosol, more preferably at least about 10 micrograms of [6]-gingerol per puff of aerosol. Alternatively, or in addition, the aerosol generated from the aerosol-generating substrate comprises up to about 25 micrograms of [6]-gingerol per puff of aerosol, preferably up to about 20 micrograms of [6]-gingerol per puff of aerosol and more preferably up to about 15 micrograms of [6]-gingerol per puff of aerosol. For example, the aerosol generated from the aerosol-generating substrate may comprise between about 0.3 micrograms and about 25 micrograms of [6]-gingerol per puff of aerosol, or between about 5 micrograms and about 20 micrograms of [6]-gingerol per puff of aerosol, or between about 10 micrograms and about 15 micrograms of [6]-gingerol per puff of aerosol.

Preferably, the aerosol according to the present invention comprises at least about 0.5 micrograms of [10]-gingerol per puff of aerosol, more preferably at least about 0.75 microgram of [10]-gingerol per puff of aerosol. Alternatively, or in addition, the aerosol generated from the aerosol-generating substrate comprises up to about 5 micrograms of [10]-gingerol per puff of aerosol, preferably up to about 3 micrograms of [10]-gingerol per puff of aerosol and more preferably up to about 2 micrograms of [10]-gingerol per puff of aerosol. For example, the aerosol generated from the aerosol-generating substrate may comprise between about 0.03 micrograms and about 5 micrograms of [10]-gingerol per puff of aerosol, or between about 0.5 micrograms and about 3 micrograms of [10]-gingerol per puff of aerosol, or between about 0.75 microgram and about 2 micrograms of [10]-gingerol per puff of aerosol.

Preferably, the aerosol according to the present invention comprises at least about 10 micrograms of [10]-shogaol per puff of aerosol, more preferably at least about 20 micrograms of [10]-shogaol per puff of aerosol. Alternatively, or in addition, the aerosol generated from the aerosol-generating substrate comprises up to about 50 micrograms of [10]-shogaol per puff of aerosol, preferably up to about 40 micrograms of [10]-shogaol per puff of aerosol and more preferably up to about 30 micrograms of [10]-shogaol per

puff of aerosol. For example, the aerosol generated from the aerosol-generating substrate may comprise between about 0.7 micrograms and about 50 micrograms of [10]-shogaol per puff of aerosol, or between about 10 micrograms and about 40 micrograms of [10]-shogaol per puff of aerosol, or between about 20 microgram and about 30 micrograms of [10]-shogaol per puff of aerosol.

Preferably, the aerosol according to the present invention comprises at least about 5 micrograms of [8]-shogaol per puff of aerosol, more preferably at least about 10 micrograms of [8]-shogaol per puff of aerosol. Alternatively, or in addition, the aerosol generated from the aerosol-generating substrate comprises up to about 25 micrograms of [8]-shogaol per puff of aerosol, preferably up to about 20 micrograms of [8]-shogaol per puff of aerosol and more preferably up to about 15 micrograms of [8]-shogaol per puff of aerosol. For example, the aerosol generated from the aerosol-generating substrate may comprise between about 0.3 micrograms and about 25 micrograms of [8]-shogaol per puff of aerosol, or between about 5 micrograms and about 20 micrograms of [8]-shogaol per puff of aerosol, or between about 10 micrograms and about 15 micrograms of [8]-shogaol per puff of aerosol.

Preferably, the aerosol according to the present invention comprises at least about 10 micrograms of [6]-shogaol per puff of aerosol, more preferably at least about 15 micrograms of [6]-shogaol per puff of aerosol. Alternatively, or in addition, the aerosol generated from the aerosol-generating substrate comprises up to about 50 micrograms of [6]-shogaol per puff of aerosol, preferably up to about 40 micrograms of [6]-shogaol per puff of aerosol and more preferably up to about 30 micrograms of [6]-shogaol per puff of aerosol. For example, the aerosol generated from the aerosol-generating substrate may comprise between about 0.6 micrograms and about 50 micrograms of [6]-shogaol per puff of aerosol, or between about 10 micrograms and about 40 micrograms of [6]-shogaol per puff of aerosol, or between about 15 microgram and about 30 micrograms of [6]-shogaol per puff of aerosol.

According to the present invention, the aerosol composition is such that the amount of [10]-shogaol per puff is at least 10 times the amount of [10]-gingerol per puff. The ratio of [10]-shogaol to [10]-gingerol in the aerosol is therefore at least 10:1.

Preferably, the amount of [10]-shogaol per puff of aerosol is at least 15 times the amount of [10]-gingerol per puff of aerosol, such that the ratio of [10]-shogaol to [10]-gingerol in the aerosol is at least 15:1. More preferably, the amount of [10]-shogaol per puff of aerosol is at least 20 times the amount of [10]-gingerol per puff of aerosol, such that the ratio of [10]-shogaol to [10]-gingerol in the aerosol is at least 20:1.

The defined ratio of [10]-shogaol to [10]-gingerol characterises an aerosol that is derived from ginger particles. In contrast, in an aerosol produced from ginger oil, the ratio of [10]-shogaol to [10]-gingerol would be significantly different, since the level of [10]-shogaol in ginger oil is at or close to zero.

Preferably, the aerosol according to the invention further comprises at least about 0.1 milligrams of aerosol former per puff of aerosol, more preferably at least about 0.2 milligrams of aerosol per puff of aerosol and more preferably at least about 0.3 milligrams of aerosol former per puff of aerosol. Preferably, the aerosol comprises up to 0.6 milligrams of aerosol former per puff of aerosol, more preferably up to 0.5 milligrams aerosol former per puff of aerosol, more preferably up to 0.4 milligrams aerosol former per puff of aerosol.

For example, the aerosol may comprise between about 0.1 milligrams and about 0.6 milligrams of aerosol former per puff of aerosol, or between about 0.2 milligrams and about 0.5 milligrams of aerosol former per puff of aerosol, or between about 0.3 milligrams and about 0.4 milligrams of aerosol former per puff of aerosol. These values are based on a puff volume of 55 millilitres, as defined above.

Suitable aerosol formers for use in the present invention are set out above.

Preferably, the aerosol produced from an aerosol-generating substrate according to the present invention further comprise at least about 2 micrograms of nicotine per puff of aerosol, more preferably at least about 20 microgram of nicotine per puff of aerosol, more preferably at least about 40 micrograms of nicotine per puff of aerosol. Preferably, the aerosol comprises up to about 200 micrograms of nicotine per puff of aerosol, more preferably up to about 150 micrograms of nicotine per puff of aerosol, more preferably up to about 75 micrograms of nicotine per puff of aerosol. For example, the aerosol may comprise between about 2 micrograms and about 200 micrograms of nicotine per puff of aerosol, or between about 20 microgram and about 150 micrograms of nicotine per puff of aerosol, or between about 40 micrograms and about 75 micrograms of nicotine per puff of aerosol. These values are based on a puff volume of 55 millilitres, as defined above. In some embodiments of the present invention, the aerosol may contain zero micrograms of nicotine.

Alternatively or in addition, the aerosol according to the present invention may optionally further comprise at least about 0.5 milligrams of a cannabinoid compound per puff of aerosol, more preferably at least about 1 milligram of a cannabinoid compound per puff of aerosol, more preferably at least about 2 milligrams of a cannabinoid compound per puff of aerosol. Preferably, the aerosol comprises up to about 5 milligrams of a cannabinoid compound per puff of aerosol, more preferably up to about 4 milligrams of a cannabinoid compound per puff of aerosol, more preferably up to about 3 milligrams of a cannabinoid compound per puff of aerosol.

For example, the aerosol may comprise between about 0.5 milligrams and about 5 milligrams of a cannabinoid compound per puff of aerosol, or between about 1 milligram and about 4 milligrams of a cannabinoid compound per puff of aerosol, or between about 2 milligrams and about 3 milligrams of a cannabinoid compound per puff of aerosol. In some embodiments of the present invention, the aerosol may contain zero micrograms of cannabinoid compound. These values are based on a puff volume of 55 millilitres, as defined above.

Preferably, the cannabinoid compound is selected from CBD and THC. More preferably, the cannabinoid compound is CBD.

Carbon monoxide may also be present in the aerosol according to the invention and may be measured and used to further characterise the aerosol. Oxides of nitrogen such as nitric oxide and nitrogen dioxide may also be present in the aerosol and may be measured and used to further characterise the aerosol.

The aerosol according to the invention comprising the characteristic compounds from the ginger particles may be formed of particles having a mass median aerodynamic diameter (MMAD) in the range of about 0.01 to 200 microns, or about 1 to 100 microns. Preferably, where the aerosol comprises nicotine as described above, the aerosol comprises particles having a MMAD in the range of about 0.1 to about 3 microns in order to optimise the delivery of nicotine from the aerosol.

The mass median aerodynamic diameter (MMAD) of an aerosol refers to the aerodynamic diameter for which half the particulate mass of the aerosol is contributed by particles with an aerodynamic diameter larger than the MMAD and half by particles with an aerodynamic diameter smaller than the MMAD. The aerodynamic diameter is defined as the diameter of a spherical particle with a density of 1 g/cm<sup>3</sup> that has the same settling velocity as the particle being characterised.

The mass median aerodynamic diameter of an aerosol according to the invention may be determined in accordance with Section 2.8 of Schaller et al., "Evaluation of the Tobacco Heating System 2.2. Part 2: Chemical composition, genotoxicity, cytotoxicity and physical properties of the aerosol," *Regul. Toxicol. and Pharmacol.*, 81 (2016) S27-S47.

Specific embodiments will be further described, by way of example only, with reference to the accompanying drawings in which:

FIG. 1 illustrates a first embodiment of a substrate of an aerosol-generating article as described herein;

FIG. 2 illustrates an aerosol-generating system comprising an aerosol-generating article and an aerosol-generating device comprising an electric heating element;

FIG. 3 illustrates an aerosol-generating system comprising an aerosol-generating article and an aerosol-generating device comprising a combustible heating element;

FIGS. 4a and 4b illustrate a second embodiment of a substrate of an aerosol-generating article as described herein;

FIG. 5 illustrates a third embodiment of a substrate of an aerosol-generating article as described herein;

FIG. 6 is a cross sectional view of filter 1050 further comprising an aerosol-modifying element, wherein

FIG. 6a illustrates the aerosol-modifying element in the form of a spherical capsule or bead within a filter plug.

FIG. 6b illustrates the aerosol-modifying element in the form of a thread within a filter plug.

FIG. 6c illustrates the aerosol-modifying element in the form of a spherical capsule within a cavity within the filter;

FIG. 7 is a cross sectional view of a plug of aerosol-generating substrate 1020 further comprising an aerosol-modifying element in the form of a bead; and

FIG. 8 illustrates an experimental set-up for collecting aerosol samples to be analysed in order to measure characteristic compounds.

FIG. 1 illustrates a heated aerosol-generating article 1000 comprising a substrate as described herein. The article 1000 comprises four elements; the aerosol-generating substrate 1020, a hollow cellulose acetate tube 1030, a spacer element 1040, and a mouthpiece filter 1050. These four elements are arranged sequentially and in coaxial alignment and are assembled by a cigarette paper 1060 to form the aerosol-generating article 1000. The article 1000 has a mouth-end 1012, which a user inserts into his or her mouth during use, and a distal end 1013 located at the opposite end of the article to the mouth end 1012. The embodiment of an aerosol-generating article illustrated in FIG. 1 is particularly suitable for use with an electrically-operated aerosol-generating device comprising a heater for heating the aerosol-generating substrate.

When assembled, the article 1000 is about 45 millimetres in length and has an outer diameter of about 7.2 millimetres and an inner diameter of about 6.9 millimetres.

The aerosol-generating substrate 1020 comprises a plug formed from a sheet of homogenised ginger material comprising ginger particles, either alone or in combination with

tobacco particles. A number of examples of a suitable homogenised ginger material for forming the aerosol-generating substrate 1020 are shown in Table 1 below (see Samples A to D). The sheet is gathered, crimped and wrapped in a filter paper (not shown) to form the plug. The sheet includes additives, including glycerol as an aerosol former.

An aerosol-generating article 1000 as illustrated in FIG. 1 is designed to engage with an aerosol-generating device in order to be consumed. Such an aerosol-generating device includes means for heating the aerosol-generating substrate 1020 to a sufficient temperature to form an aerosol. Typically, the aerosol-generating device may comprise a heating element that surrounds the aerosol-generating article 1000 adjacent to the aerosol-generating substrate 1020, or a heating element that is inserted into the aerosol-generating substrate 1020.

Once engaged with an aerosol-generating device, a user draws on the mouth-end 1012 of the smoking article 1000 and the aerosol-generating substrate 1020 is heated to a temperature of about 375 degrees Celsius. At this temperature, volatile compounds are evolved from the aerosol-generating substrate 1020. These compounds condense to form an aerosol. The aerosol is drawn through the filter 1050 and into the user's mouth.

FIG. 2 illustrates a portion of an electrically-operated aerosol-generating system 2000 that utilises a heating blade 2100 to heat an aerosol-generating substrate 1020 of an aerosol-generating article 1000. The heating blade is mounted within an aerosol article receiving chamber of an electrically-operated aerosol-generating device 2010. The aerosol-generating device defines a plurality of air holes 2050 for allowing air to flow to the aerosol-generating article 1000. Air flow is indicated by arrows on FIG. 2. The aerosol-generating device comprises a power supply and electronics, which are not illustrated in FIG. 2. The aerosol-generating article 1000 of FIG. 2 is as described in relation to FIG. 1.

In an alternative configuration shown in FIG. 3, the aerosol-generating system is shown with a combustible heating element. While the article 1000 of FIG. 1 is intended to be consumed in conjunction with an aerosol-generating device, the article 1001 of FIG. 3 comprises a combustible heat source 1080 that may be ignited and transfer heat to the aerosol-generating substrate 1020 to form an inhalable aerosol. The combustible heat source 80 is a charcoal element that is assembled in proximity to the aerosol-generating substrate at a distal end 13 of the rod 11. Elements that are essentially the same as elements in FIG. 1 have been given the same numbering.

FIGS. 4a and 4b illustrate a second embodiment of a heated aerosol-generating article 4000a, 4000b. The aerosol-generating substrate 4020a, 4020b comprises a first downstream plug 4021 formed from of particulate plant material comprising primarily ginger particles, and a second upstream plug 4022 formed from particulate plant material comprising primarily tobacco particles. A suitable homogenised plant material for use in the first downstream plug is shown in Table 1 below as Sample A. A suitable homogenised tobacco material for use in the second upstream plug is shown in Table 1 below as Sample E. Sample E comprises only tobacco particles and is included for the purposes of comparison only.

In each of the plugs, the homogenised plant material is in the form of sheets, which are crimped and wrapped in a filter paper (not shown). The sheets both include additives, including glycerol as an aerosol former. In the embodiment

shown in FIG. 4a, the plugs are combined in an abutting end to end relationship to form the rod and are of equal length of about 6 mm each. In a more preferred embodiment (not shown), the second plug is preferably longer than the first plug, for example, preferably 2 mm longer, more preferably 3 mm longer, such that the second plug is 7 or 7.5 mm in length while the first plug is 5 or 4.5 mm in length, to provide a desired ratio of tobacco to ginger particles in the substrate. In FIG. 4b, the cellulose acetate tube support element 1030 has been omitted.

The article 4000a, 4000b, analogously to the article 1000 in FIG. 1, is particularly suitable for use with the electrically-operated aerosol-generating system 2000 comprising a heater shown in FIG. 2. Elements that are essentially the same elements in FIG. 1 have been given the same numbering. It may be envisaged by the skilled person that a combustible heat source (not shown) may be instead be used with the second embodiment in lieu of the electrical heating element, in a configuration similar to the configuration containing combustible heat source 1080 in article 1001 of FIG. 3.

FIG. 5 illustrates a third embodiment of a heated aerosol-generating article 5000. The aerosol-generating substrate 5020 comprises a rod formed from a first sheet of homogenised ginger material formed of particulate plant material comprising primarily ginger particles, and a second sheet of homogenised tobacco material comprising primarily cast-leaf tobacco. A suitable homogenised ginger material for use as the first sheet is shown in Table 1 below as Sample A. A suitable homogenised tobacco material for use as the second sheet is shown in Table 1 below as Sample E.

The second sheet overlies the first sheet, and the combined sheets have been crimped, gathered and at least partially wrapped in a filter paper (not shown) to form a plug that is part of the rod. Both sheets include additives, including glycerol as an aerosol former. The article 5000, analogously to the article 1000 in FIG. 1, is particularly suitable for use with the electrically-operated aerosol-generating system 2000 comprising a heater shown in FIG. 2. Elements that are essentially the same elements in FIG. 1 have been given the same numbering. It may be envisaged by the skilled person that a combustible heat source (not shown) may be instead be used with the third embodiment in lieu of the electrical heating element, in a configuration similar to the configuration containing combustible heat source 1080 in article 1001 of FIG. 3.

FIG. 6 is a cross sectional view of filter 1050 further comprising an aerosol-modifying element. In FIG. 6a, the filter 1050 further comprises an aerosol-modifying element in the form of a spherical capsule or bead 605.

In the embodiment of FIG. 6a, the capsule or bead 605 is embedded in the filter segment 601 and is surrounded on all sides by the filter material 603. In this embodiment, the capsule comprises an outer shell and an inner core, and the inner core contains a liquid flavourant. The liquid flavourant is for flavouring aerosol during use of the aerosol-generating article provided with the filter. The capsule 605 releases at least a portion of the liquid flavourant when the filter is subjected to external force, for example by squeezing by a consumer. In the embodiment shown, the capsule is generally spherical, with a substantially continuous outer shell containing the liquid flavourant.

In the embodiment of FIG. 6b, the filter segment 601 comprises a plug of filter material 603 and a central flavour-bearing thread 607 that extends axially through the plug of filter material 603 parallel to the longitudinal axis of the filter 1050. The central flavour-bearing thread 607 is of

substantially the same length as the plug of filter material 603, so that the ends of the central flavour-bearing thread 607 are visible at the ends of the filter segment 601. In FIG. 6b, filter material 603 is cellulose acetate tow. The central flavour-bearing thread 607 is formed from twisted filter plug wrap and loaded with an aerosol-modifying agent.

In the embodiment of FIG. 6c, the filter segment 601 comprises more than one plug of filter material 603, 603'. Preferably, the plugs of filter material 603, 603' are formed from cellulose acetate, such that they are able to filter the aerosol provided by the aerosol generating article. A wrapper 609 is wrapped around and connects filter plugs 603, 603'. Inside a cavity 611 is a capsule 605 comprising an outer shell and an inner core, and the inner core contains a liquid flavourant. The capsule is otherwise similar to the embodiment of FIG. 6a.

FIG. 7 is a cross sectional view of aerosol-generating substrate 1020 further comprising an aerosol-modifying element in the form of a bead 705. The aerosol-generating substrate 1020 comprises a plug 703 formed from a sheet of homogenised ginger material comprising tobacco particles and ginger particles. The flavour delivery material in the bead 705 incorporates a flavourant which is released upon heating the material to a temperature above 220 degrees Celsius. The flavourant is therefore released into the aerosol as a portion of the plug is heated during use.

## EXAMPLE

Different samples of homogenised plant material for use in an aerosol-generating substrate according to the invention, as described above with reference to the figures, were prepared from aqueous slurries having compositions shown Table 1. Samples A to D comprise ginger particles in accordance with the invention. Sample E comprises only tobacco particles and is included for the purposes of comparison only.

The particulate plant material in all samples accounts for 75 percent of the dry weight of the homogenised plant material, with glycerol, guar gum and cellulose fibres accounting for the remaining 25 percent of the dry weight of homogenised plant material. The samples are prepared from an aqueous slurry containing between 78-79 kg of water per 100 kg of slurry.

In the table below, % DWB refers to the "dry weight base," in this case, the percent by weight calculated relative to the dry weight of the homogenised plant material. The ginger powder was formed from *Zingiber officinale* roots which were dried and ground to a final D95=130 microns by triple impact milling.

TABLE 1

| Sample | Dry content of slurries |                 |                  |                  |                          |
|--------|-------------------------|-----------------|------------------|------------------|--------------------------|
|        | Ginger powder (% DWB)   | Tobacco (% DWB) | Glycerol (% DWB) | Guar Gum (% DWB) | Cellulose fibres (% DWB) |
| A      | 75                      | 0               | 18               | 3                | 4                        |
| B      | 15                      | 60              | 18               | 3                | 4                        |
| C      | 7.5                     | 67.5            | 18               | 3                | 4                        |
| D      | 2.5                     | 72.5            | 18               | 3                | 4                        |
| E      | 0                       | 75              | 18               | 3                | 4                        |

The slurries may be casted using a casting bar (0.6 mm) on a glass plate, dried in an oven at 140 degrees Celsius for 7 minutes, and then dried in a second oven at 120 degrees Celsius for 30 seconds.

For each of the samples A to E of homogenised plant material, a plug was produced from a single continuous sheet of the homogenised plant material, the sheets each having widths of between 100 mm to 125 mm. The individual sheets had thickness of about 220 microns and a grammage of about 200 g/m<sup>2</sup>. The cut width of each sheet was adapted based on the thickness of each sheet to produce rods of comparable volume. The sheets were crimped to a height of 165 microns to 170 microns, and rolled into plugs having a length of about 12 mm and diameters of about 7 mm, circumscribed by a paper wrapper.

For each of the plugs, an aerosol-generating article having an overall length of about 45 mm was formed having a structure as shown in FIG. 3 comprising, from the downstream end: a mouth end cellulose acetate filter (about 7 mm long), an aerosol spacer comprising a crimped sheet of polylactic acid polymer (about 18 mm long), a hollow acetate tube (about 8 mm long) and the plug of aerosol-generating substrate.

For Sample A of homogenised ginger material, for which ginger particles make up 100 percent of the particulate plant material, the characteristic compounds were extracted from the plug of homogenised ginger material using methanol as detailed above. The extract was analysed as described above to confirm the presence of the characteristic compounds and to measure the amounts of the characteristic compounds. The results of this analysis are shown below in Table 2, wherein the amounts indicated correspond to the amount per aerosol-generating article, wherein the aerosol-generating substrate of the aerosol-generating article contained 233 mg of the Sample A of homogenised ginger material. For the purposes of comparison, the amounts of the characteristic compound present in the particulate plant material (ginger particles) used to form Sample A are also shown. For the particulate plant material, the amounts indicated correspond to the amount of the characteristic compound in a sample of particulate plant material having a weight corresponding to the total weight of the particulate plant material in the aerosol-generating article containing 233 mg of Sample A.

TABLE 2

| Amount of ginger-specific compounds in the particulate plant material and in the aerosol-generating substrate |                                                                     |                                                                   |
|---------------------------------------------------------------------------------------------------------------|---------------------------------------------------------------------|-------------------------------------------------------------------|
| Characteristic Compound                                                                                       | Amount in the aerosol-generating substrate (micrograms per article) | Amount in the particulate plant material (micrograms per article) |
| [6]-gingerol                                                                                                  | 79.1                                                                | 97.4                                                              |
| [10]-gingerol                                                                                                 | 733.8                                                               | 990.1                                                             |
| [10]-shogaol                                                                                                  | 542.2                                                               | 629.7                                                             |
| [6]-shogaol                                                                                                   | 659.1                                                               | 698.1                                                             |
| [8]-shogaol                                                                                                   | 229.2                                                               | 252.3                                                             |

For each of the samples B to D comprising a proportion of ginger particles, the amount of the characteristic compounds can be estimated based on the values in Table 2 by assuming that the amount is present in proportion to the weight of the ginger particles.

Mainstream aerosols of the aerosol-generating articles incorporating aerosol-generating substrates formed from Samples A to E of homogenised plant material were generated in accordance with Test Method A, as defined above. For each sample, the aerosol that was produced was trapped and analysed.

As described in detail above, according to Test Method A, the aerosol-generating articles were tested using the commercially available IQOS® heat-not-burn device tobacco

heating system 2.2 holder (THS2.2 holder) from Philip Morris Products S.A. The aerosol-generating articles were heated under a Health Canada machine-smoking regimen over 30 puffs with a puff volume of 55 ml, puff duration of 2 seconds and a puff interval of 30 seconds (as described in ISO/TR 19478-1:2014).

The aerosol generated during the smoking test was collected on a Cambridge filter pad and extracted with a liquid solvent. FIG. 10 shows suitable apparatus for generating and collecting the aerosol from the aerosol-generating articles.

Aerosol-generating device 111 shown in FIG. 10 is a commercially available tobacco heating device (IQOS). The contents of the mainstream aerosol generated during the Health Canada smoking test as detailed above are collected in aerosol collection chamber 113 on aerosol collection line 120. Glass fibre filter pad 140 is a 44 mm Cambridge glass fibre filter pad (CFP) in accordance with ISO 4387 and ISO 3308.

For LC-HRAM-MS Analysis:

Extraction solvent 170, 170a, which in this case is methanol and internal standard (ISTD) solution, is present at a volume of 10 mL in each micro-impinger 160, 160a. The cold baths 161, 161a each contain a dry ice-isopropyl ether to maintain the micro-impingers 160, 160a each at approximately -60° C. The gas-vapour phase is trapped in the extraction solvent 170, 170a as the aerosol bubbles through micro-impingers 160, 160a. The combined solutions from the two micro-impingers are isolated as impinger-trapped gas-vapor phase solution 180 in step 181.

The CFP and the impinger-trapped gas-vapor phase solution 180 are combined in a clean Pyrex® tube in step 190. In step 200, the total particulate matter is extracted from the CFP using the impinger-trapped gas-vapor phase solution 180 (which contains methanol as a solvent) by thoroughly shaking (disintegrating the CFP), vortexing for 5 min and finally centrifuging (4500 g, 5 min, 10° C.). Aliquots (300 µL) of the reconstituted whole aerosol extract 220 were transferred into a silanized chromatographic vial and diluted with methanol (700 µL), since the extraction solvent 170, 170a already comprised internal standard (ISTD) solution. The vials were closed and mixed for 5 minutes using an Eppendorf ThermoMixer (5° C.; 2000 rpm).

Aliquots (1.5 µL) of the diluted extracts were injected and analyzed by LC-HRAM-MS in both full scan mode and data-dependent fragmentation mode for compound identification.

For GCxGC-TOFMS Analysis:

As discussed above, when samples for GCxGC-TOFMS experiments are prepared, different solvents are suitable for extracting and analysing polar compounds, non-polar compounds and volatile compounds separated from whole aerosol. The experimental set-up is identical to that described with respect to sample collection for LC-HRAM-MS, with the exceptions indicated below.

55 Nonpolar & Polar

Extraction solvent 171, 171a, is present at a volume of 10 mL and is an 80:20 v/v mixture of dichlormethane and methanol, also containing retention-index marker (RIM) compounds and stable isotopically labeled internal standards (ISTD). The cold baths 162, 162a each contain a dry ice-isopropanol mixture to maintain the micro-impingers 160, 160a each at approximately -78° C. The gas-vapour phase is trapped in the extraction solvent 171, 171a as the aerosol bubbles through micro-impingers 160, 160a. The combined solutions from the two micro-impingers are isolated as impinger-trapped gas-vapor phase solution 210 in step 182.

## Nonpolar

The CFP and the impinger-trapped gas-vapor phase solution **210** are combined in a clean Pyrex® tube in step **190**. In step **200**, the total particulate matter is extracted from the CFP using the impinger-trapped gas-vapor phase solution **210** (which contains dichloromethane and methanol as a solvent) by thoroughly shaking (disintegrating the CFP), vortexing for 5 min and finally centrifuging (4500 g, 5 min, 10° C.) to isolate the polar and non-polar components of the whole aerosol extract **230**.

In step **250**, an 10 mL aliquot **240** of the whole aerosol extract **230** was taken. In step **260**, a 10 mL aliquot of water is added, and the entire sample is shaken and centrifuged. The non-polar fraction **270** was separated, dried with sodium sulfate and analysed by GCxGC-TOFMS in full scan mode.

## Polar

ISTD and RIM compounds were added to polar fraction **280**, which was then directly analysed by GCxGC-TOFMS in full scan mode.

Each smoking replicate (n=3) comprises the accumulated trapped and reconstituted non-polar fraction **270** and polar fraction **280** for each sample

## Volatile Components

Whole aerosol was trapped using two micro-impingers **160**, **160a** in series. Extraction solvent **172**, **172a**, which in this case is N,N-dimethylformamide (DMF) containing retention-index marker (RIM) compounds and stable isotopically labeled internal standards (ISTD), is present at a volume of 10 mL in each micro-impinger **160**, **160a**. The cold baths **161**, **161a** each contain a dry ice-isopropyl ether to maintain the micro-impingers **160**, **160a** each at approximately -60° C. The gas-vapor phase is trapped in the extraction solvent **170**, **170a** as the aerosol bubbles through micro-impingers **160**, **160a**. The combined solutions from the two micro-impingers are isolated as a volatile-containing phase **211** in step **183**. The volatile-containing phase **211** is analysed separately from the other phases and injected directly into the GCxGC-TOFMS using cool-on-column injection without further preparation.

Table 3 below shows the levels of the characteristic compounds from the ginger particles in the aerosol generated from an aerosol-generating article incorporating Sample A of homogenised ginger material, including ginger particles only. For the purposes of comparison, Table 3 also shows the levels of the characteristic compounds in the aerosol generated from an aerosol-generating article incorporating Sample E of homogenised tobacco material, including tobacco particles only (and therefore not in accordance with the invention).

TABLE 3

| Compound      | Content of characteristic compounds in aerosol |                                      |                                            |                                         |
|---------------|------------------------------------------------|--------------------------------------|--------------------------------------------|-----------------------------------------|
|               | Sample A<br>(micrograms<br>per article)        | Sample A<br>(micrograms<br>per gram) | Sample A<br>(micrograms<br>per 55 ml puff) | Sample E<br>(micrograms<br>per article) |
| [6]-gingerol  | 132.2                                          | 495.1                                | 11.02                                      | 0.6                                     |
| [10]-gingerol | 11                                             | 41.2                                 | 0.92                                       | 0.0                                     |
| [10]-shogaol  | 257                                            | 962.5                                | 21.42                                      | 0.8                                     |
| [6]-shogaol   | 222.4                                          | 833                                  | 18.53                                      | 0.4                                     |
| [8]-shogaol   | 130.4                                          | 488.4                                | 10.87                                      | 0.7                                     |

In the aerosol generated from Sample A, relatively high levels of the characteristic compounds were measured. The ratio of [10]-shogaol to [10]-gingerol was above 20:1. The levels of the characteristic compounds was therefore indica-

tive of the presence of ginger particles in the sample. In contrast, for the tobacco only Sample E, which contained substantially no ginger particles, the levels of the characteristic compounds were found to be at or close to zero.

For each of the samples B to D comprising a proportion of ginger particles, the amount of the characteristic compounds in the aerosol can be estimated based on the values in Table 3 by assuming that the amount is present in proportion to the weight of the ginger particles in the aerosol-generating substrate from which the aerosol is generated.

Table 4 below shows more generally the composition of the aerosol generated from the aerosol-generating article incorporating the Sample A (ginger only) compared to the composition of the aerosol generated from the tobacco only Sample E (tobacco only). The reduction indicated is the reduction provided by replacing the tobacco particles in the homogenised tobacco material of Sample E with ginger particles.

As shown in Table 4, the aerosol produced by Sample A containing 100 percent by weight ginger powder based on the dry weight of the particulate plant material results in reduced levels of propionaldehyde, crotonaldehyde, methylethylketone, acetaldehyde, phenol, o-cresol, catechol, hydroquinone, acrylonitrile, styrene, isoprene, pyridine, benzo[a]pyrene, benz[a]anthracene, and total particulate matter when compared to the level of the aerosol in Sample E produced using 100 percent by weight tobacco based on the dry weight of the particulate plant material.

TABLE 4

|    | Composition of aerosol                |          |          |           |
|----|---------------------------------------|----------|----------|-----------|
|    | Aerosol Constituent                   | Sample E | Sample A | Reduction |
| 35 | Nicotine (mg/article)                 | 1.25     | 0        | -100%     |
|    | Glycerol (mg/article)                 | 4.6      | 3.5      | -24%      |
|    | Total particulate matter (mg/article) | 49.9     | 36.3     | -27%      |
| 40 | Carbon monoxide (mg/article)          | 0.53     | 1.11     | 108%      |
|    | Propionaldehyde (µg/article)          | 12.7     | 13.7     | -7%       |
|    | Crotonaldehyde (µg/article)           | 1.7      | 1.9      | -11%      |
| 45 | Methyl ethyl ketone (µg/article)      | 6.5      | 5.1      | -21%      |
|    | Acetaldehyde (µg/article)             | 192.9    | 176.5    | -9%       |
|    | Phenol (µg/article)                   | 1.5      | 0.13     | -91%      |
| 50 | o-cresol (µg/article)                 | 0.0798   | 0.0256   | -68%      |
|    | Catechol (µg/article)                 | 13.8     | 6.3      | -54%      |
|    | Hydroquinone (µg/article)             | 6.7      | 1.2      | -83%      |
|    | Acrylonitrile (µg/article)            | 0.160    | 0.114    | -29%      |
| 55 | Styrene (µg/article)                  | 0.560    | 0.355    | -37%      |
|    | Isoprene (µg/article)                 | 1.823    | 0.351    | -81%      |
|    | Pyridine (µg/article)                 | 7.36     | 1.59     | -78%      |
|    | Benzo[a]pyrene (µg/article)           | 0.79     | <0.054   | -93%      |
|    | Benz[a]anthracene (µg/article)        | 1.88     | <0.047   | -98%      |

60 The invention claimed is:

1. An aerosol-generating article, comprising:  
an aerosol-generating substrate comprising

a homogenised ginger material comprising ginger par-

ticles, tobacco particles, an aerosol former, and a binder;

at least 10 micrograms of [6]-gingerol per gram of the aerosol-generating substrate, on a dry weight basis;

- at least 90 micrograms of [10]-gingerol per gram of the aerosol-generating substrate, on a dry weight basis; at least 70 micrograms of [10]-shogaol per gram of the aerosol-generating substrate, on a dry weight basis; at least 30 micrograms of [8]-shogaol per gram of the aerosol-generating substrate, on a dry weight basis; and at least 80 micrograms of [6]-shogaol per gram of the aerosol-generating substrate, on a dry weight basis.
2. The aerosol-generating article according to claim 1, wherein the amount of [6]-shogaol per gram of the aerosol-generating substrate is at least 5 times the amount of [10]-gingerol per gram of the aerosol-generating substrate.
3. The aerosol-generating article according to claim 1, wherein the aerosol-generating substrate further comprises between 1 milligram and 20 milligrams of nicotine per gram of the aerosol-generating substrate, on a dry weight basis.
4. The aerosol-generating article according to claim 1, wherein the homogenised ginger material comprises between 5 percent by weight and 30 percent by weight of aerosol former and between 1 percent by weight and 10 percent by weight of binder, on a dry weight basis.
5. The aerosol-generating article according to claim 1, wherein the binder comprises guar gum.
6. The aerosol-generating article according to claim 1, wherein the homogenised ginger material further comprises at least 2.5 percent by weight of the ginger particles, on a dry weight basis.
7. The aerosol-generating article according to claim 1, wherein a weight ratio of the ginger particles to the tobacco particles is no more than 1:4.
8. The aerosol-generating article according to claim 1, wherein the homogenised ginger material in the aerosol-generating substrate is in the form of cast leaf.
9. The aerosol-generating article according to claim 1, wherein the homogenised ginger material in the aerosol-generating substrate is in the form of ginger paper.
10. The aerosol-generating article according to claim 1, wherein upon heating of the aerosol-generating substrate according to Test Method A, an aerosol is generated comprising:
- at least 15 micrograms of [6]-gingerol per gram of the aerosol-generating substrate, on a dry weight basis; at least 1.5 micrograms of [10]-gingerol per gram of the aerosol-generating substrate, on a dry weight basis; at least 30 micrograms of [10]-shogaol per gram of the aerosol-generating substrate, on a dry weight basis; at least 15 micrograms of [8]-shogaol per gram of the aerosol-generating substrate, on a dry weight basis; and at least 30 micrograms of [6]-shogaol per gram of the aerosol-generating substrate, on a dry weight basis, wherein the amount of [10]-shogaol per gram of the aerosol-generating substrate is at least 10 times the amount of [10]-gingerol per gram of the aerosol-generating substrate.
11. The aerosol-generating article according to claim 10, wherein the amount of [10]-shogaol per gram of the substrate is at least 20 times the amount of [10]-gingerol per gram of the substrate.
12. The aerosol-generating article according to claim 1, wherein upon heating of the aerosol-generating substrate

- according to Test Method A, an aerosol generated from the aerosol-generating substrate comprises:
- [6]-gingerol in an amount of at least 0.3 micrograms per puff of the aerosol; [10]-gingerol in an amount of at least 0.03 micrograms per puff of the aerosol; [10]-shogaol in an amount of at least 0.7 micrograms per puff of the aerosol; [8]-shogaol in an amount of at least 0.3 micrograms per puff of the aerosol; and [6]-shogaol in an amount of at least 0.6 micrograms per puff of the aerosol, wherein a puff of the aerosol has a volume of 55 millilitres as generated by a smoking machine, and wherein the amount of [10]-shogaol per puff is at least 10 times the amount of [10]-gingerol per puff.
13. An aerosol-generating system, comprising:
- an aerosol-generating device comprising a heating element; and
- an aerosol-generating article according to claim 1.
14. An aerosol-generating substrate, comprising:
- a homogenised ginger material comprising ginger particles, tobacco particles, an aerosol former, and a binder; at least 10 micrograms of [6]-gingerol per gram of the aerosol-generating substrate, on a dry weight basis; at least 90 micrograms of [10]-gingerol per gram of the aerosol-generating substrate, on a dry weight basis; at least 70 micrograms of [10]-shogaol per gram of the aerosol-generating substrate, on a dry weight basis; at least 30 micrograms of [8]-shogaol per gram of the aerosol-generating substrate, on a dry weight basis; and at least 80 micrograms of [6]-shogaol per gram of the aerosol-generating substrate, on a dry weight basis.
15. An aerosol produced upon heating of an aerosol-generating substrate according to claim 14, the aerosol comprising:
- [6]-gingerol in an amount of at least 0.3 micrograms per puff of the aerosol; [10]-gingerol in an amount of at least 0.03 micrograms per puff of the aerosol; [10]-shogaol in an amount of at least 0.7 micrograms per puff of the aerosol; [8]-shogaol in an amount of at least 0.3 micrograms per puff of the aerosol; and [6]-shogaol in an amount of at least 0.6 micrograms per puff of the aerosol, wherein a puff of the aerosol has a volume of 55 millilitres as generated by a smoking machine, and wherein the amount of [10]-shogaol per puff is at least 10 times the amount of [10]-gingerol per puff.
16. A method of making an aerosol-generating substrate according to claim 14, the method comprising the steps of:
- forming a slurry comprising ginger particles, tobacco particles, water, an aerosol former, an exogenous binder; casting or extruding the slurry in the form of a sheet or strands; and drying the sheet or strands at between 80 degrees Celsius and 160 degrees Celsius.